

# United States Patent [19]

Wey

[11] 4,399,215  
[45] Aug. 16, 1983

- [54] **DOUBLE-JET PRECIPITATION PROCESSES AND PRODUCTS THEREOF**
- [75] Inventor: **Jong-Shinn Wey**, Penfield, N.Y.
- [73] Assignee: **Eastman Kodak Company**, Rochester, N.Y.
- [21] Appl. No.: **429,403**
- [22] Filed: **Sep. 30, 1982**

## Related U.S. Application Data

- [63] Continuation-in-part of Ser. No. 320,908, Nov. 12, 1981, abandoned.
- [51] Int. Cl.<sup>3</sup> ..... G03C 1/02; G03C 5/26
- [52] U.S. Cl. ..... 430/567; 430/569
- [58] Field of Search ..... 430/567, 569

## [56] References Cited

### U.S. PATENT DOCUMENTS

- 3,784,381 1/1974 Perignon .  
4,063,951 12/1977 Bogg .  
4,067,739 1/1978 Lewis .  
4,150,994 4/1979 Maternaghan .  
4,184,877 1/1980 Maternaghan .  
4,184,878 1/1980 Maternaghan .

### FOREIGN PATENT DOCUMENTS

- 2905655 2/1979 Fed. Rep. of Germany .  
2921077 5/1979 Fed. Rep. of Germany .  
55-142329 11/1980 Japan .  
1570581 7/1980 United Kingdom .

### OTHER PUBLICATIONS

- Claes et al., "Crystal Habit Modification of AgCl by Impurities Determining the Solvation," *The Journal of Photographic Science*, vol. 21 pp. 39-50, 1973.
- Wyrscz, "Sulfur Sensitization of Monosized Silver Chloride Emulsions with (111), (110) and (100) Crystal

Habit", Paper III-13, International Congress of Photographic Science pp. 122-124, 1978.

Grundlagen der Photographische Prozesse mit Silberhalogeniden Band 2, Die Photographische Emulsion und die Verarbeitung Photographischer Schichten, Akademische Verlagsgesellschaft Frankfurt AM Main (1968) p. 639.

Symposium: Torino 1963, *Photographic Science*, Edited by C. Semerano and U. Mazzucato, Focal Press, pp. 52-55.

Gutoff, "Nucleation and Growth Rates During the Precipitation of Silver Halide Photographic Emulsions," *Photographic Science and Engineering*, vol. 14, No. 4, Jul.-Aug. 1970, pp. 248-250.

deCugnac and Chateau, "Evolution of the Morphology of Silver Bromide Crystals During Physical Ripening," *Science et Industries Photographiques*, vol. 33, No. 2 (1962) pp. 121-125.

Duffin, *Photographic Emulsion Chemistry*, Focal Press, 1966, pp. 66-72.

Trivelli and Smith, "The Effect of Silver Iodide Upon the Structure of Bromo-Iodide Precipitation Series," *The Photographic Journal*, vol. LXXX, Jul. 1940, pp. 285-288.

Primary Examiner—M. F. Downey  
Attorney, Agent, or Firm—Carl O. Thomas

## [57] ABSTRACT

A double-jet precipitation process is disclosed for preparing radiation-sensitive photographic emulsions containing tabular silver chloride grains which are substantially internally free of bromide and iodide. In forming the emulsions chloride and silver salt solutions are concurrently run into a dispersing medium while controlling both pH and pAg. Tabular grains having an average aspect ratio of greater than 8:1 are obtained.

17 Claims, 5 Drawing Figures



*FIG. 1*



*FIG. 2*



*FIG. 3*



*FIG. 4*



FIG. 5

## DOUBLE-JET PRECIPITATION PROCESSES AND PRODUCTS THEREOF

This is a continuation-in-part of copending, commonly assigned U.S. Ser. No. 320,908, filed Nov. 12, 1981, now abandoned.

### FIELD OF THE INVENTION

The present invention is drawn to improved double-jet precipitation processes and products thereof. More specifically, the invention is drawn to an improvement in double-jet processes of preparing radiation-sensitive photographic emulsions by concurrently introducing chloride and silver salt solutions into a dispersing medium as well as to the photographic emulsions produced by these processes.

### BACKGROUND OF THE INVENTION

Radiation-sensitive silver chloride photographic emulsions are known to offer specific advantages. For example, silver chloride exhibits less native sensitivity to the visible portion of the spectrum than other photographically useful silver halides. Further, silver chloride is more soluble than other photographically useful silver halides, thereby permitting development and fixing to be achieved in shorter times.

It is well recognized in the art that silver chloride strongly favors the formation of crystals having {100} crystal faces. In the overwhelming majority of photographic emulsions silver chloride crystals when present are in the form of cubic grains. With some difficulty it has been possible to modify the crystal habit of silver chloride. Claes et al., "Crystal Habit Modification of AgCl by Impurities Determining the Solvation", *The Journal of Photographic Science*, Vol. 21, pp. 39-50, 1973, teaches the formation of silver chloride crystals with {110} and {111} faces through the use of various grain growth modifiers. Wyrscz, "Sulfur Sensitization of Monosized Silver Chloride Emulsions with {111}, {110} and {100} Crystal Habit", Paper III-13, *International Congress of Photographic Science*, pp. 122-124, 1978, discloses a triple-jet precipitation process in which silver chloride is precipitated in the presence of ammonia and small amounts of divalent cadmium ions. In the presence of cadmium ions control of pAg and pH resulted in the formation of rhombododecahedral {110}, octahedral {111}, and cubic {100} crystal habits.

Tabular silver bromide grains have been extensively studied, often in macro-sizes having no photographic utility. Tabular grains are herein defined as those having two substantially parallel crystal faces, each of which is substantially larger than any other single crystal face of the grain. The term "substantially parallel" as used herein is intended to include surfaces that appear parallel on direct or indirect visual inspection at 10,000 times magnification. The aspect ratio—that is, the ratio of diameter to thickness—of tabular grains is substantially greater than 1:1. High aspect ratio tabular grain silver bromide emulsions were reported by deCugnac and Chateau, "Evolution of the Morphology of Silver Bromide Crystals During Physical Ripening", *Science et Industries Photographiques*, Vol. 33, No. 2 (1962), pp. 121-125.

From 1937 until the 1950's the Eastman Kodak Company sold a Duplitized® radiographic film product under the name No-Screen X-Ray Code 5133. The product contained as coatings on opposite major faces

of a film support sulfur sensitized silver bromide emulsions. Since the emulsions were intended to be exposed by X-radiation, they were not spectrally sensitized. The tabular grains had an average aspect ratio in the range of from about 5 to 7:1. The tabular grains accounted for greater than 50% of the projected area while nontabular grains accounted for greater than 25% of the projected area. The emulsion having the highest average aspect ratio, chosen from several remakes, had an average tabular grain diameter of 2.5 microns, an average tabular grain thickness of 0.36 micron, and an average aspect ratio of 7:1. In other remakes the emulsions contained thicker, smaller diameter tabular grains which were of lower average aspect ratio.

Although tabular grain silver bromoiodide emulsions are known in the art, none exhibit a high average aspect ratio. A discussion of tabular silver bromoiodide grains appears in Duffin, *Photographic Emulsion Chemistry*, Focal Press, 1966, pp. 66-72, and Trivelli and Smith, "The Effect of Silver Iodide Upon the Structure of Bromo-Iodide Precipitation Series", *The Photographic Journal*, Vol. LXXX, July 1940, pp. 285-288. Trivelli and Smith observed a pronounced reduction in both grain size and aspect ratio with the introduction of iodide. Gutoff, "Nucleation and Growth Rates During the Precipitation of Silver Halide Photographic Emulsions," *Photographic Sciences and Engineering*, Vol. 14, No. 4, July-August 1970, pp. 248-257, reports preparing silver bromide and silver bromoiodide emulsions of the type prepared by single-jet precipitations using a continuous precipitation apparatus.

It has been recognized that advantages in covering power and other photographic characteristics can be obtained by preparing silver halide emulsions in which the grains are tabular—that is, areally extended in two dimensions as compared to their thickness. Bogg U.S. Pat. No. 4,063,951 teaches forming silver halide crystals of tabular habit bounded by {100} cubic faces and having an aspect ratio (based on edge length) of from 1.5 to 7:1 by a double-jet precipitation technique in which pAg is controlled within the range of from 5.0 to 7.0. As shown in FIG. 3 of Bogg, the silver halide grains formed exhibit square and rectangular major surfaces characteristic of {100} crystal faces. Lewis U.S. Pat. No. 4,067,739 teaches the preparation of monosize silver halide emulsions wherein most of the crystals are of the twinned octahedral type by forming seed crystals, causing the seed crystals to increase the size by Ostwald ripening in the presence of a silver halide solvent, and completing grain growth without renucleation or Ostwald ripening while controlling pBr (the negative logarithm of bromide ion concentration). Lewis does not mention silver chloride. Maternaghan U.S. Pat. Nos. 4,150,994 and 4,184,877, U.K. Pat. No. 1,570,581, and German OLS publications, 2,905,655 and 2,921,077 teach the formation of silver halide grains of flat twinned octahedral configuration by employing seed crystals which are at least 90 mole percent iodide. (Except as otherwise indicated, all references to halide percentages are based on silver present in the corresponding emulsion, grain, or grain region being discussed; e.g., a grain consisting of silver bromoiodide containing 40 mole percent iodide also contains 60 mole percent bromide.) Japanese Pat. No. Kokai No. 142,329, published Nov. 6, 1980, appears to be essentially cumulative with Maternaghan, but is not restricted to the use of silver iodide seed grains.

Perignon U.S. Pat. No. 3,784,381 teaches the preparation of silver chloroiodide and silver chlorobromoiodide emulsions by precipitating the silver halide grains at a pH in the range of from 5 to 9 and a pAg of at least about 7.8 by adding to the precipitation mixture no later than at the end of the precipitation a weak solvent for silver halide selected from the group consisting of ammonium chloride, ammonium nitrate, and magnesium chloride.

Wilgus and Haefner U.S. Ser. No. 429,420, filed concurrently herewith and commonly assigned, titled *HIGH ASPECT RATIO SILVER BROMOIODIDE EMULSIONS AND PROCESSES FOR THEIR PREPARATION*, which is a continuation-in-part of U.S. Ser. No. 320,905, filed Nov. 12, 1981, now abandoned, discloses high aspect ratio silver bromoiodide emulsions and a process for their preparation.

Kofron et al U.S. Ser. No. 429,407, filed concurrently herewith and commonly assigned, titled *SENSITIZED HIGH ASPECT RATIO SILVER HALIDE EMULSIONS AND PHOTOGRAPHIC ELEMENTS*, which is a continuation-in-part of U.S. Ser. No. 320,904, filed Nov. 12, 1981, now abandoned, discloses chemically and spectrally sensitized high aspect ratio tabular grain silver halide emulsions and photographic elements incorporating these emulsions. Kofron et al discloses that photographic elements can exhibit improved sharpness and exhibit a wider separation between their speed in a spectral region of intrinsic sensitivity and a spectrally sensitized region. Kofron et al further discloses speed-granularity advantages for high aspect ratio tabular grain silver bromoiodide emulsions.

Daubendiek and Strong U.S. Ser. No. 429,587, filed concurrently herewith and commonly assigned, titled *AN IMPROVED PROCESS FOR THE PREPARATION OF HIGH ASPECT RATIO SILVER BROMOIODIDE EMULSIONS*, which is a continuation-in-part of U.S. Ser. No. 320,906, filed Nov. 12, 1981, now abandoned, discloses an improvement on the processes of Maternaghan whereby high aspect ratio tabular grain silver bromoiodide emulsions can be prepared.

Abbott and Jones U.S. Ser. No. 430,222, filed concurrently herewith and commonly assigned, titled *RADIOGRAPHIC ELEMENTS EXHIBITING REDUCED CROSSOVER*, which is a continuation-in-part of U.S. Ser. No. 320,907, filed Nov. 12, 1981, now abandoned, discloses the use of spectrally sensitized high aspect ratio tabular grain emulsions in radiographic elements coated on both major surfaces of a radiation transmitting support to control crossover. Comparisons of radiographic elements containing high aspect ratio tabular grain emulsions with similar radiographic elements containing conventional emulsions show that reduced crossover can be attributed to the high aspect ratio tabular grain emulsions. Alternatively, comparable crossover levels can be achieved with reduced silver coverages and/or improved speed-granularity relationships.

#### SUMMARY OF THE INVENTION

In one aspect this invention is directed to a radiation-sensitive photographic emulsion comprising a dispersing medium and silver chloride grains, wherein at least 50 percent of the total projected area of the silver chloride is provided by tabular grains which are substantially internally free of both iodide and bromide, have an average aspect ratio greater than 8:1, and have opposed, substantially parallel {111} major crystal faces.

In another aspect this invention is directed to an improvement in a double-jet precipitation process of preparing a radiation-sensitive photographic emulsion comprised of a dispersing medium and silver halide grains which are substantially internally free of iodide and bromide by concurrently introducing chloride and silver salt solutions into the dispersing medium in the presence of ammonia. The improvement comprises, while concurrently introducing the chloride and silver salt solutions, maintaining the pAg within the dispersing medium in the range of from 6.5 to 10 and maintaining the pH within the dispersing medium in the range of from 8 to 10, thereby precipitating at least 50 percent, based on total grain projected area, of the silver chloride grains in the form of tabular grains having an average aspect ratio of greater than 8:1 and having opposed, substantially parallel {111} major crystal faces.

In an additional aspect, this invention is directed to a photographic element comprised of a support and at least one radiation-sensitive emulsion layer comprised of a radiation-sensitive emulsion as described above.

Prior to this invention there has been a need for photographic emulsions which provide the specific advantages of both silver chloride and grain configurations of relatively high aspect ratio—that is, greater than 8:1. The present invention satisfies this need. The improved silver chloride emulsions of this invention can produce further photographic advantages, such as higher maximum density and higher covering power. Still other photographic advantages can be realized, depending upon the specific photographic application contemplated.

In addition, the present invention offers an advantageous method of preparing these and other silver halide grains of relatively high aspect ratio which are internally free of silver iodide and silver bromide. In one preferred form the present invention is directed to substantially pure silver chloride emulsions of relatively high aspect ratio and to their preparation. The precipitation process does not require the use of cadmium dopants or organic grain growth modifiers to establish grain morphology. Although not incompatible with the practice of this invention, it is unnecessary to either provide seed crystals or to vary precipitation conditions between the nucleation and growth stages of emulsion precipitation in order to obtain grains of high aspect ratios. In its preferred form, the precipitation process of this invention is then manipulatively simpler than the prior art processes of obtaining silver halide grains of high aspect ratios.

The advantages taught by Kofron et al, cited above, in photographic elements and Abbott and Jones, cited above, in radiographic elements can be realized when high aspect ratio tabular grain emulsions according to the present invention are employed. Further, the advantages taught by Jones and Hill, U.S. Ser. No. 430,092, filed concurrently herewith and commonly assigned, titled *PHOTOGRAPHIC IMAGE TRANSFER FILM UNIT*, which is a continuation-in-part of U.S. Ser. No. 320,911, filed Nov. 12, 1981, now abandoned can be realized with the emulsions of the present invention incorporated in the disclosed image transfer film units. The image transfer film units are capable of achieving a higher performance ratio of photographic speed to silver coverage (i.e., silver halide coated per unit area), faster access to a viewable transferred image, and higher contrast of transferred images with less time of development.

This invention can be better appreciated by reference to the detailed description of the preferred embodiments which follows when considered in conjunction with the drawings.

#### BRIEF DESCRIPTION OF THE DRAWINGS

FIGS. 1 through 4 are photomicrographs of silver halide emulsions.

FIG. 5 is a schematic diagram illustrating considerations relevant to scattering of exposing radiation.

#### DESCRIPTION OF PREFERRED EMBODIMENTS

The radiation-sensitive emulsions of the present invention are comprised of a dispersing medium and silver chloride tabular grains which are substantially internally free of both bromide and iodide. To obtain the advantages of tabular grains, it is preferred that the grains be relatively thin and have a relatively high aspect ratio. As employed herein the term "aspect ratio" refers to the ratio of the diameter of the grain to its thickness. The "diameter" of the grain is in turn defined as the diameter of a circle having an area equal to the projected area of the grain as viewed in a photomicrograph of an emulsion sample. The term "projected area" is used in the same sense as the terms "projection area" and "projective area" commonly employed in the art; see, for example, James and Higgins, *Fundamentals of Photographic Theory*, Morgan and Morgan, New York, p. 15. The tabular grains of the present invention have an average aspect ratio of greater than 8:1 and preferably have an average aspect ratio of at least 10:1. Under optimum conditions of preparation aspect ratios of 20:1 or higher are contemplated. As will be apparent, the thinner the grains, the higher their aspect ratio for a given diameter. Typically grains of desirable aspect ratios are those having an average thickness of less than 0.80 micron. Typically the tabular grains have a thickness of at least 0.10 micron, although even thinner tabular grains can in principle be prepared.

Of the silver chloride grains in the emulsions according to the present invention, at least 50 percent, preferably at least 75 percent, based on the total projected area of the grains, are present in the form of tabular grains. The tabular grains have opposed, substantially parallel {111} major crystal faces, typically of triangular or truncated triangular configuration. Surprisingly, the tabular grains appear to have the same configuration as are generally observed for tabular grains of silver bromide and silver bromoiodide. That is, both the major faces and the edges of the tabular grains in the emulsions of this invention appear to be bounded by {111} crystal faces.

The silver chloride tabular grains according to this invention are substantially internally free of bromide and iodide. Alternatively stated, the tabular grains consist essentially of silver chloride as initially formed. The presence of even small amounts of bromide during grain formation interferes with the formation of the desired tabular configuration. If iodide is present during silver chloride grain formation, it tends to reduce the aspect ratios obtained and results in the formation of a higher proportion of nontabular grains.

The requirement that the tabular grains internally consist essentially of silver chloride does not preclude the presence of bromide and/or iodide in the tabular grains. Once tabular silver chloride grains have been formed according to the process of the present invention,

other halides can be incorporated into the grains by procedures well known to those skilled in the art. Techniques for forming silver salt shells are illustrated by Berriman U.S. Pat. No. 3,367,778, Porter et al U.S. Pat. Nos. 3,206,313 and 3,317,322, Morgan U.S. Pat. No. 3,917,485, and Maternaghan, cited above. Since conventional techniques for shelling do not favor the formation of high aspect ratio tabular grains, as shell growth proceeds the average aspect ratio of the emulsion declines. If conditions favorable for tabular grain formation are present in the reaction vessel during shell formation, shell growth can occur preferentially on the outer edges of the grains so that aspect ratio need not decline. Wey and Wilgus U.S. Ser. No. 431,855, filed concurrently herewith and commonly assigned, titled *NOVEL SILVER CHLOROBROMIDE EMULSIONS AND PROCESSES FOR THEIR PREPARATION*, which is a continuation-in-part of U.S. Ser. No. 920,899, filed Nov. 12, 1981, now abandoned both here incorporated by reference, specifically teaches procedures for precipitating silver chlorobromide in annular regions of tabular grains without necessarily reducing the aspect ratios of the resulting grains. The tabular grain regions containing silver, chloride, and bromide are formed by maintaining a molar ratio of chloride and bromide ions of from 1.6 to about 260:1 and the total concentration of halide ions in the reaction vessel in the range of from 0.10 to 0.90 normal during introduction of silver, chloride, bromide, and, optionally, iodide salts into the reaction vessel. The molar ratio of silver chloride to silver bromide in the tabular grains can range from 1:99 to 2:3. Evans, Daubendiek, and Raleigh U.S. Ser. No. 431,912, filed concurrently herewith and commonly assigned, titled *DIRECT REVERSAL EMULSIONS AND PHOTOGRAPHIC ELEMENTS USEFUL IN IMAGE TRANSFER FILM UNITS*, which is a continuation-in-part of U.S. Ser. No. 320,891, filed Nov. 12, 1981, now abandoned both here incorporated by reference, specifically discloses the preparation of high aspect ratio core-shell tabular grain emulsions for use in forming direct reversal images.

By adding both halide and silver salts after the silver chloride tabular grains are formed, the original grains remain intact, but serve as nuclei for the deposition of additional silver halide. The resulting tabular grains remain substantially internally free of both bromide and iodide ions. If bromide and/or iodide salts are added to the emulsion containing tabular silver chloride grains without the addition of silver salt, the heavier halides will displace chloride in the silver chloride crystal structure. Displacement begins at the crystal surfaces and progresses toward the interior of the grains. The substitution of chloride ions in the silver chloride crystal lattice with bromide ions and, optionally, a minor proportion of iodide ions is well known. Such emulsions are referred to in the art as halide-converted silver halide emulsions. Techniques for preparing halide-converted emulsions and uses therefor are illustrated by Knott et al U.S. Pat. No. 2,456,953, Davey et al U.S. Pat. No. 2,592,250, MacWilliam U.S. Pat. No. 2,756,148, and Evans U.S. Pat. No. 3,622,318. In the present invention less than 20 mole percent, preferably less than 10 percent, of the halide is introduced by displacement. At high levels of displacement the tabular configuration of the grains is degraded or even destroyed. Thus, while substitution of bromide and/or iodide ions for chloride ions at or near the grain surfaces are contemplated, massive halide conversions, as are

common in producing internal latent image forming grains, are not contemplated in the practice of this invention.

In the formation of tabular silver chloride grains according to this invention an aqueous dispersing medium is placed in a conventional silver halide reaction vessel. The pH and pAg of the dispersing medium within the reaction vessel are adjusted to satisfy the conditions of precipitation according to this invention. (As herein employed, pH, pCl, and pAg are defined as the negative logarithm of hydrogen, chloride, and silver ion concentration, respectively.) Since the ranges of pAg values contemplated for use in the practice of this invention are on the halide side of the equivalence point (the pAg at which the concentration of silver and halide ions are stoichiometrically equal), a small amount of an aqueous chloride salt solution is employed to adjust pAg initially. Thereafter, an aqueous silver salt solution and aqueous chloride salt solution are concurrently run into the reaction vessel. The pAg within the reaction vessel is maintained within the desired limits by conventional measurement techniques and by adjusting the relative flow rates of the silver and chloride salt solutions. Using conventional sensing techniques, the pH in the reaction vessel is also monitored and is maintained within a predetermined range by the addition of a base while the silver and chloride salts are being introduced. Apparatus and techniques for controlling pAg and pH during silver halide precipitation are disclosed by Oliver U.S. Pat. No. 3,031,304, Culhane et al U.S. Pat. No. 3,821,002, and Claes and Peelaers, *Photographische Korrespondenz*, 103, 161 (1967).

It is believed that the presence of a ripening agent—specifically, ammonia, plays a role in the formation of tabular silver chloride grains according to this invention. It has been found convenient to supply aqueous ammonia hydroxide to the reaction vessel to satisfy the pH requirements of the precipitation process. As is generally recognized, ammonia is present in an equilibrium relationship in aqueous ammonium hydroxide solutions. The ammonium hydroxide in the aqueous solution can result from the direct addition of ammonium hydroxide or from the addition of a water soluble ammonium salt, such as ammonium chloride or ammonium nitrate, and a strong base, such as an alkali hydroxide, e.g., sodium or potassium hydroxide. The ammonium hydroxide is preferably added to the reaction vessel through a third jet concurrently with the addition of silver and halide salts. Alternatively the ammonium hydroxide can be combined with either the aqueous silver or halide salt solutions during addition.

Useful tabular silver chloride emulsions can be formed according to the present invention by maintaining pAg values in the range of from 6.5 to 10 (preferably 7.0 to 9.4) and pH values in the range of from 8 to 10 (preferably 8.5 to 9.7) at conventional silver chloride precipitation temperatures below about 60° C. Higher conventional precipitation temperatures can, of course, be employed, but provide tabular grains of larger size. In an optimum mode of practicing this invention pAg is maintained in the reaction vessel in the range of from 7.6 to 8.9 while ammonium hydroxide is introduced into the reaction vessel in an amount sufficient to maintain pH in the range of from 8.8 to 9.5 while introducing the chloride salt solution. The temperature of the reaction vessel is optimally maintained in the range of from 20° to 40° C.

At least 50 percent, based on grain projected area, of the silver chloride precipitated by the process described above is in the form of tabular grains. Preferably at least 75 percent of the total grain projected area is in the form of tabular grains. Although minor amounts of nontabular grains are fully compatible with many photographic applications, to achieve the full advantages of tabular grains the proportion of tabular grains can be increased. Larger tabular silver chloride grains can be mechanically separated from smaller, nontabular grains in a mixed population of grains using conventional separation techniques—e.g., by using a centrifuge or a hydrocyclone. An illustrative teaching of hydrocyclone separation is provided by Audran et al U.S. Pat. No. 3,326,641.

Except as specifically described above, the process of preparing a tabular grain silver chloride emulsion can take various conventional forms. The aqueous silver salt solution can employ a soluble silver salt, such as silver nitrate, while the aqueous chloride salt solution can employ one or more water soluble ammonium, alkali metal (e.g., sodium or potassium), or alkaline earth metal (e.g., magnesium or calcium) chloride salts. The aqueous silver and chloride salt solutions can vary widely in concentrations, ranging from 0.1 to 7.0 molar or even higher.

In addition to running silver and chloride salts into the reaction vessel, a variety of other compounds are known to be useful when present in the reaction vessel during silver halide precipitation. For example, minor concentrations of compounds of metals such as copper, thallium, lead, bismuth, cadmium, gold, and Group VIII noble metals, can be present during precipitation of the silver halide emulsion, as illustrated by Arnold et al U.S. Pat. No. 1,195,432, Hochstetter U.S. Pat. No. 1,951,933, Trivelli et al U.S. Pat. No. 2,448,060, Overman U.S. Pat. No. 2,628,167, Mueller et al U.S. Pat. No. 2,950,972, sidebotham U.S. Pat. No. 3,488,709, Rosecrants et al U.S. Pat. No. 3,737,313, and *Research Disclosure*, Vol. 134, June 1975, Item 13452. Distribution of the metal dopants in the silver chloride grains can be controlled by selective placement of the metal compounds in the reaction vessel or by controlled addition during the introduction of silver and chloride salts.

The individual silver and halide salts can be added to the reaction vessel through surface or subsurface delivery tubes by gravity feed or by delivery apparatus for maintaining control of the rate of delivery and the pH, pCl, and/or pAg of the reaction vessel contents, as illustrated by Culhane et al U.S. Pat. No. 3,821,002, Oliver U.S. Pat. No. 3,031,304 and Claes et al, *Photographische Korrespondenz*, Band 102, No. 10, 1967, p. 162. In order to obtain rapid distribution of the reactants within the reaction vessel, specially constructed mixing devices can be employed, as illustrated by Audran U.S. Pat. No. 2,996,287, McCrossen et al U.S. Pat. No. 3,342,605, Frame et al U.S. Pat. No. 3,415,650, Porter et al U.S. Pat. No. 3,785,777, Finnicum et al U.S. Pat. No. 4,147,551, Verhille et al U.S. Pat. No. 4,171,224, Calamur U.K. patent application No. 2,022,431A, Saito et al German OLS Nos. 2,555,364 and 2,556,885, and *Research Disclosure*, Volume 166, February 1978, Item 16662. *Research Disclosure* and its predecessor, *Product Licensing Index*, are publications of Industrial Opportunities Ltd.; Homewell, Havant; Hampshire, P09 1EF, United Kingdom.

In forming the tabular grain silver chloride emulsions peptizer concentrations of from 0.2 to about 10 percent

by weight, based on the total weight of emulsion components in the reaction vessel, can be employed; it is preferred to keep the concentration of the peptizer in the reaction vessel prior to and during grain formation below about 6 percent by weight, based on the total weight. It is common practice to maintain the concentration of the peptizer in the reaction vessel below about 6 percent, based on the total weight, prior to and during silver halide formation and to adjust the emulsion vehicle concentration upwardly for optimum coating characteristics by delayed, supplemental vehicle additions. It is contemplated that the emulsion as initially formed will contain from about 5 to 50 grams of peptizer per mole of silver halide, preferably about 10 to 30 grams of peptizer per mole of silver halide. Additional vehicle can be added later to bring the concentration up to as high as 1000 grams per mole of silver halide. Preferably the concentration of vehicle in the finished emulsion is above 50 grams per mole of silver halide. When coated and dried in forming a photographic element the vehicle preferably forms about 30 to 70 percent by weight of the emulsion layer.

Vehicles (which include both binders and peptizers) can be chosen from among those conventionally employed in silver halide emulsions. Preferred peptizers are hydrophilic colloids, which can be employed alone or in combination with hydrophobic materials. Suitable hydrophilic materials include substances such as proteins, protein derivatives, cellulose derivatives—e.g., cellulose esters, gelatin—e.g., alkali-treated gelatin (cattle bone or hide gelatin) or acid-treated gelatin (pigskin gelatin), gelatin derivatives—e.g., acetylated gelatin, phthalated gelatin and the like, polysaccharides such as dextran, gum arabic, zein, casein, pectin, collagen derivatives, agar-agar, arrowroot, albumin and the like as described in Yutzy et al U.S. Pat. Nos. 2,614,928 and '929, Lowe et al U.S. Pat. Nos. 2,691,582, 2,614,930, '931, 2,327,808 and 2,448,534, Gates et al U.S. Pat. Nos. 2,787,545 and 2,956,880, Himmelmann et al U.S. Pat. No. 3,061,436, Farrell et al U.S. Pat. No. 2,816,027, Ryan U.S. Pat. Nos. 3,132,945, 3,138,461 and 3,186,846, Dersch et al U.K. Pat. No. 1,167,159 and U.S. Pat. Nos. 2,960,405 and 3,436,220, Geary U.S. Pat. No. 3,486,896, Gazzard U.K. Pat. No. 793,549, Gates et al U.S. Pat. Nos. 2,992,213, 3,157,506, 3,184,312 and 3,539,353, Miller et al U.S. Pat. No. 3,227,571, Boyer et al U.S. Pat. No. 3,532,502, Malan U.S. Pat. No. 3,551,151, Lohmer et al U.S. Pat. No. 4,018,609, Luciani et al U.K. Pat. No. 1,186,790, Hori et al U.K. Pat. No. 1,489,080 and Belgian Pat. No. 856,631, U.K. Pat. No. 1,490,644, U.K. Pat. No. 1,483,551, Arase et al U.K. Pat. No. 1,459,906, Salo U.S. Pat. Nos. 2,110,491 and 2,311,086, Fallesen U.S. Pat. No. 2,343,650, Yutzy U.S. Pat. No. 2,322,085, Lowe U.S. Pat. No. 2,563,791, Talbot et al U.S. Pat. No. 2,725,293, Hilborn U.S. Pat. No. 2,748,022, DePauw et al U.S. Pat. No. 2,956,883, Ritchie U.K. Pat. No. 2,095, DeStubner U.S. Pat. No. 1,752,069, Sheppard et al U.S. Pat. No. 2,127,573, Lierg U.S. Pat. No. 2,256,720, Gaspar U.S. Pat. No. 2,361,936, Farmer U.K. Pat. No. 15,727, Stevens U.K. Pat. No. 1,062,116 and Yamamoto et al U.S. Pat. No. 3,923,517.

Other materials commonly employed in combination with hydrophilic colloid peptizers as vehicles (including vehicle extenders—e.g., materials in the form of latices) include synthetic polymeric peptizers, carriers and/or binders such as poly(vinyl lactams), acrylamide polymers, polyvinyl alcohol and its derivatives, polyvinyl acetals, polymers of alkyl and sulfoalkyl acrylates

and methacrylates, hydrolyzed polyvinyl acetates, polyamides, polyvinyl pyridine, acrylic acid polymers, maleic anhydride copolymers, polyalkylene oxides, methacrylamide copolymers, polyvinyl oxazolidinones, maleic acid copolymers, vinylamine copolymers, methacrylic acid copolymers, acryloyloxyalkylsulfonic acid copolymers, sulfoalkylacrylamide copolymers, polyalkyleneimine copolymers, polyamines, N,N-dialkylaminoalkyl acrylates, vinyl imidazole copolymers, vinyl sulfide copolymers, halogenated styrene polymers, amineacrylamide polymers, polypeptides and the like as described in Hollister et al U.S. Pat. Nos. 3,679,425, 3,706,564 and 3,813,251, Lowe U.S. Pat. Nos. 2,253,078, 2,276,322, '323, 2,281,703, 2,311,058 and 2,414,207, Lowe et al U.S. Pat. Nos. 2,484,456, 2,541,474 and 2,632,704, Perry et al U.S. Pat. No. 3,425,836, Smith et al U.S. Pat. Nos. 3,415,653 and 3,615,624, Smith U.S. Pat. No. 3,488,708, Whiteley et al U.S. Pat. Nos. 3,392,025 and 3,511,818, Fitzgerald U.S. Pat. Nos. 3,681,079, 3,721,565, 3,852,073, 3,861,918 and 3,925,083, Fitzgerald et al U.S. Pat. No. 3,879,205, Nottorf U.S. Pat. No. 3,142,568, Houck et al U.S. Pat. Nos. 3,062,674 and 3,220,844, Dann et al U.S. Pat. No. 2,882,161, Schupp U.S. Pat. No. 2,579,016, Weaver U.S. Pat. No. 2,829,053, Alles et al U.S. Pat. No. 2,698,240, Priest et al U.S. Pat. No. 3,003,879, Merrill et al U.S. Pat. No. 3,419,397, Stonham U.S. Pat. No. 3,284,207, Lohmer et al U.S. Pat. No. 3,167,430, Williams U.S. Pat. No. 2,957,767, Dawson et al U.S. Pat. No. 2,893,867, Smith et al U.S. Pat. Nos. 2,860,986 and 2,904,539, Ponticello et al U.S. Pat. Nos. 3,929,482 and 3,860,428, Ponticello U.S. Pat. No. 3,939,130, Dykstra U.S. Pat. No. 3,411,911 and Dykstra et al Canadian Pat. No. 774,054, Ream et al U.S. Pat. No. 3,287,289, Smith U.K. Pat. No. 1,466,600, Stevens U.K. Pat. No. 1,062,116, Fordyce U.S. Pat. No. 2,211,323, Martinez U.S. Pat. No. 2,284,877, Watkins U.S. Pat. No. 2,420,455, Jones U.S. Pat. No. 2,533,166, Bolton U.S. Pat. No. 2,495,918, Graves U.S. Pat. No. 2,289,775, Yackel U.S. Pat. No. 2,565,418, Unruh et al U.S. Pat. Nos. 2,865,893 and 2,875,059, Rees et al U.S. Pat. No. 3,536,491, Broadhead et al U.K. Pat. No. 1,348,815, Taylor et al U.S. Pat. No. 3,479,186, Merrill et al U.S. Pat. No. 3,520,857, Bacon et al U.S. Pat. No. 3,690,888, Bowman U.S. Pat. No. 3,748,143, Dickinson et al U.K. Pat. Nos. 808,227 and '228, Wood U.K. Pat. No. 822,192 and Iguchi et al U.K. Pat. No. 1,398,055. These additional materials need not be present in the reaction vessel during silver halide precipitation, but rather are conventionally added to the emulsion prior to coating. The vehicle materials, including particularly the hydrophilic colloids, as well as the hydrophobic materials useful in combination therewith can be employed not only in the emulsion layers of the photographic elements of this invention, but also in other layers, such as overcoat layers, interlayers and layers positioned beneath the emulsion layers.

It is specifically contemplated that grain ripening can occur during the precipitation of emulsions according to the present invention. Silver chloride, by reason of its higher level of solubility, is influenced to a lesser extent than other silver halides by ripening agents. Known silver halide solvents are useful in promoting ripening. For example, ripening agents can be entirely contained within the dispersing medium in the reaction vessel before silver and halide salt addition, or they can be introduced into the reaction vessel along with one or more of the halide salt, silver salt, or peptizer. In still

another variant the ripening agent can be introduced independently during halide and silver salt additions.

The tabular grain high aspect ratio emulsions of the present invention are preferably washed to remove soluble salts. The soluble salts can be removed by decantation, filtration, and/or chill setting and leaching, as illustrated by Craft U.S. Pat. No. 2,316,845 and McFall et al U.S. Pat. No. 3,396,027; by coagulation washing, as illustrated by Hewitson et al U.S. Pat. No. 2,618,556, Yutzy et al U.S. Pat. No. 2,614,928, Yackel U.S. Pat. No. 2,565,418, Hart et al U.S. Pat. No. 3,241,969, Waller et al U.S. Pat. No. 2,489,341, Klinger U.K. Pat. No. 1,305,409 and Dersch et al U.K. Pat. No. 1,167,159; by centrifugation and decantation of a coagulated emulsion, as illustrated by Murray U.S. Pat. No. 2,463,794, 15 Ujihara et al U.S. Pat. No. 3,707,378, Audran U.S. Pat. No. 2,996,287 and Timson U.S. Pat. No. 3,498,454; by employing hydrocyclones alone or in combination with centrifuges, as illustrated by U.K. Pat. No. 1,336,692, Claes U.K. Pat. No. 1,356,573 and Ushomirskii et al 20 Soviet Chemical Industry, Vol. 6, No. 3, 1974, pp. 181-185; by diafiltration with a semipermeable membrane, as illustrated by Research Disclosure, Vol. 102, October 1972, Item 10208, Hagemayer et al Research Disclosure, Vol. 131, March 1975, Item 13122, Bonnet 25 Research Disclosure, Vol. 135, July 1975, Item 13477, Berg et al German OLS No. 2,436,461, Bolton U.S. Pat. No. 2,495,918, and Mignot U.S. Pat. No. 4,334,012 commonly assigned and here incorporated by reference, or by employing an ion exchange resin, as illustrated by 30 Maley U.S. Pat. No. 3,782,953 and Noble U.S. Pat. No. 2,827,428. The emulsions, with or without sensitizers, can be dried and stored prior to use as illustrated by Research Disclosure, Vol. 101, September 1972, Item 10152. In the present invention washing is particularly 35 advantageous in terminating ripening of the tabular grains after the completion of precipitation to avoid increasing their thickness and reducing their aspect ratio.

The high aspect ratio tabular grain silver halide emulsions of the present invention are chemically sensitized as taught by Kofron et al, cited above. They can be chemically sensitized with active gelatin, as illustrated by T. H. James, *The Theory of the Photographic Process*, 4th Ed., Macmillan, 1977, pp. 67-76, or with sulfur, 40 selenium, tellurium, gold, platinum, palladium, iridium, osmium, rhodium, rhenium, or phosphorus sensitizers or combinations of these sensitizers, such as at pAg levels of from 5 to 10, pH levels of from 5 to 8 and temperatures of from 30° to 80° C., as illustrated by Research Disclosure, Vol. 120, April 1974, Item 12008, Research Disclosure, Vol. 134, June 1975, Item 13452, Sheppard et al U.S. Pat. No. 1,623,499, Matthies et al U.S. Pat. No. 1,673,522, Waller et al U.S. Pat. No. 2,399,083, Damschroder et al U.S. Pat. No. 2,642,361, 45 McVeigh U.S. Pat. No. 3,297,447, Dunn U.S. Pat. No. 3,297,446, McBride U.K. Pat. No. 1,315,755, Berry et al U.S. Pat. No. 3,772,031, Gilman et al U.S. Pat. No. 3,761,267, Ohi et al U.S. Pat. No. 3,857,711, Klinger et al U.S. Pat. No. 3,565,633, Oftedahl U.S. Pat. Nos. 3,901,714 and 3,904,415 and Simons U.K. Pat. No. 1,396,696; chemical sensitization being optionally conducted in the presence of thiocyanate compounds, as described in Damschroder U.S. Pat. No. 2,642,361; sulfur containing compounds of the type disclosed in Lowe et al U.S. Pat. No. 2,521,926, Williams et al U.S. Pat. No. 3,021,215, and Bigelow U.S. Pat. No. 4,054,457. It is specifically contemplated to sensitize 50

chemically in the presence of finish (chemical sensitization) modifiers—that is, compounds known to suppress fog and increase speed when present during chemical sensitization, such as azaindenes, azapyridazines, azapyrimidines, benzothiazolium salts, and sensitizers having heterocyclic nuclei. Exemplary finish modifiers are described in Brooker et al U.S. Pat. No. 2,131,038, Dostes U.S. Pat. No. 3,411,914, Kuwabara et al U.S. Pat. No. 3,554,757, Oguchi et al U.S. Pat. No. 3,565,631, Oftedahl U.S. Pat. No. 3,901,714, Walworth Canadian Pat. No. 778,723, and Duffin *Photographic Emulsion Chemistry*, Focal Press (1966), New York, pp. 138-143. Additionally or alternatively, the emulsions can be reduction sensitized—e.g., with hydrogen, as illustrated by Janusonis U.S. Pat. No. 3,891,446 and Babcock et al U.S. Pat. No. 3,984,249, by low pAg (e.g., less than 5) and/or high pH (e.g., greater than 8) treatment or through the use of reducing agents, such as stannous chloride, thiourea dioxide, polyamines and aminebo酣anes, as illustrated by Allen et al U.S. Pat. No. 2,983,609, Oftedahl et al *Research Disclosure*, Vol. 136, August 1975, Item 13654, Lowe et al U.S. Pat. Nos. 2,518,698 and 2,739,060, Roberts et al U.S. Pat. Nos. 2,743,182 and '183, Chambers et al U.S. Pat. No. 3,026,203 and Bigelow et al U.S. Pat. No. 3,361,564. Surface chemical sensitization, including sub-surface sensitization, illustrated by Morgan U.S. Pat. No. 3,917,485 and Becker U.S. Pat. No. 3,966,476, is specifically contemplated.

Although the high aspect ratio tabular grain silver halide emulsions of the present invention are generally responsive to the techniques for chemical sensitization known in the art in a qualitative sense, in a quantitative sense—that is, in terms of the actual speed increases realized—the tabular grain emulsions require careful investigation to identify the optimum chemical sensitization for each individual emulsion, certain preferred embodiments being more specifically discussed below.

In addition to being chemically sensitized the high aspect ratio tabular grain silver chloride emulsions of the present invention are also spectrally sensitized. It is specifically contemplated to employ spectral sensitizing dyes that exhibit absorption maxima in the blue and minus blue—i.e., green and red, portions of the visible spectrum. In addition, for specialized applications, spectral sensitizing dyes can be employed which improve spectral response beyond the visible spectrum. For example, the use of infrared absorbing spectral sensitizers is specifically contemplated.

The emulsions of this invention can be spectrally sensitized with dyes from a variety of classes, including the polymethine dye class, which includes the cyanines, merocyanines, complex cyanines and merocyanines (i.e., tri-, tetra- and poly-nuclear cyanines and merocyanines), oxonols, hemioxonols, styryls, merostyryls and streptocyanines.

The cyanine spectral sensitizing dyes include, joined by a methine linkage, two basic heterocyclic nuclei, such as those derived from quinolinium, pyridinium, isoquinolinium, 3H-indolium, benz[e]indolium, oxazolium, oxazolinium, thiazolium, thiazolinium, selenazolium, selenazolinium, imidazolium, imidazolinium, benzoxazolium, benzothiazolium, benzoselenazolium, benzimidazolium, naphthoxazolium, naphthothiazolium, naphthoselenazolium, dihydronaphthothiazolium, pyrylium, and imidazopyrazinium quaternary salts.

The merocyanine spectral sensitizing dyes include, joined by a methine linkage, a basic heterocyclic nucleus of the cyanine dye type and an acidic nucleus, such as can be derived from barbituric acid, 2-thiobarbituric acid, rhodanine, hydantoin, 2-thiohydantoin, 4-thiohydantoin, 2-pyrazolin-5-one, 2-isoxazolin-5-one, indan-1,3-dione, cyclohexane-1,3-dione, 1,3-dioxane-4,6-dione, pyrazolin-3,5-dione, pentane-2,4-dione, alkylsulfonylacetonitrile, malononitrile, isoquinolin-4-one, and chroman-2,4-dione.

One or more spectral sensitizing dyes may be used. Dyes with sensitizing maxima at wavelengths throughout the visible spectrum and with a great variety of spectral sensitivity curve shapes are known. The choice and relative proportions of dyes depends upon the region of the spectrum to which sensitivity is desired and upon the shape of the spectral sensitivity curve desired. Dyes with overlapping spectral sensitivity curves will often yield in combination a curve in which the sensitivity at each wavelength in the area of overlap is approximately equal to the sum of the sensitivities of the individual dyes. Thus, it is possible to use combinations of dyes with different maxima to achieve a spectral sensitivity curve with a maximum intermediate to the sensitizing maxima of the individual dyes.

Combinations of spectral sensitizing dyes can be used which result in supersensitization—that is, spectral sensitization that is greater in some spectral region than that from any concentration of one of the dyes alone or that which would result from the additive effect of the dyes. Supersensitization can be achieved with selected combinations of spectral sensitizing dyes and other addenda, such as stabilizers and antifoggants, development accelerators or inhibitors, coating aids, brighteners and antistatic agents. Any one of several mechanisms as well as compounds which can be responsible for supersensitization are discussed by Gilman, "Review of the Mechanisms of Supersensitization", *Photographic Science and Engineering*, Vol. 18, 1974, pp. 418-430.

Spectral sensitizing dyes also affect the emulsions in other ways. Spectral sensitizing dyes can also function as antifoggants or stabilizers, development accelerators or inhibitors, and halogen acceptors or electron acceptors, as disclosed in Brooker et al U.S. Pat. No. 2,131,038 and Shiba et al U.S. Pat. No. 3,930,860.

Sensitizing action can be correlated to the position of molecular energy levels of a dye with respect to ground state and conduction band energy levels of the silver halide crystals. These energy levels can in turn be correlated to polarographic oxidation and reduction potentials, as discussed in *Photographic Science and Engineering*, Vol. 18, 1974, pp. 49-53 (Sturmer et al), pp. 175-178 (Leubner) and pp. 475-485 (Gilman). Oxidation and reduction potentials can be measured as described by R. J. Cox, *Photographic Sensitivity*, Academic Press, 1973, Chapter 15.

The chemistry of cyanine and related dyes is illustrated by Weissberger and Taylor, *Special Topics of Heterocyclic Chemistry*, John Wiley and Sons, New York, 1977, Chapter VIII; Venkataraman, *The Chemistry of Synthetic Dyes*, Academic Press, New York, 1971, Chapter V; James, *The Theory of the Photographic Process*, 4th Ed., Macmillan, 1977, Chapter 8, and F. M. Hamer, *Cyanine Dyes and Related Compounds*, John Wiley and Sons, 1964.

Among useful spectral sensitizing dyes for sensitizing silver halide emulsions are those found in U.K. Pat. No.

- 742,112, Brooker U.S. Pat. Nos. 1,846,300, '301, '302, '303, '304, 2,078,233 and 2,089,729, Brooker et al U.S. Pat. Nos. 2,165,338, 2,213,238, 2,231,658, 2,493,747, '748, 2,526,632, 2,739,964 (Reissue No. 24,292), 5 2,778,823, 2,917,516, 3,352,857, 3,411,916 and 3,431,111, Wilmanns et al U.S. Pat. No. 2,295,276, Sprague U.S. Pat. Nos. 2,481,698 and 2,503,776, Carroll et al U.S. Pat. Nos. 2,688,545 and 2,704,714, Larive et al U.S. Pat. No. 2,921,067, Jones U.S. Pat. No. 2,945,763, Nys et al U.S. 10 Pat. No. 3,282,933, Schwan et al U.S. Pat. No. 3,397,060, Riester U.S. Pat. No. 3,660,102, Kampfer et al U.S. Pat. No. 3,660,103, Taber et al U.S. Pat. Nos. 3,335,010, 3,352,680 and 3,384,486, Lincoln et al U.S. Pat. No. 3,397,981, Fumia et al U.S. Pat. Nos. 3,482,978 15 and 3,623,881, Spence et al U.S. Pat. No. 3,718,470 and Mee U.S. Pat. No. 4,025,349. Examples of useful dye combinations, including supersensitizing dye combinations, are found in Motter U.S. Pat. No. 3,506,443 and Schwan et al U.S. Pat. No. 3,672,898. As examples of 20 supersensitizing combinations of spectral sensitizing dyes and non-light absorbing addenda, it is specifically contemplated to employ thiocyanates during spectral sensitization, as taught by Leermakers U.S. Pat. No. 2,221,805; bis-triazinylaminostilbenes, as taught by McFall et al U.S. Pat. No. 2,933,390; sulfonated aromatic compounds, as taught by Jones et al U.S. Pat. No. 2,937,089; mercapto-substituted heterocycles, as taught by Riester U.S. Pat. No. 3,457,078; iodide, as taught by U.K. Pat. No. 1,413,826; and still other compounds, such as those disclosed by Gilman, "Review of the Mechanisms of Supersensitization," cited above. (It should be noted that when iodide is employed to improve spectral sensitization, it can displace halide present in the crystal lattice at the grain surface, thereby converting the grains to silver haloiodide grains.)

Conventional amounts of dyes can be employed in spectrally sensitizing the emulsion layers containing nontabular silver halide grains. To realize the full advantages of this invention it is preferred to adsorb spectral sensitizing dye to the tabular grain surfaces in a substantially optimum amount—that is, in an amount sufficient to realize at least 60 percent of the maximum photographic speed attainable from the grains under contemplated conditions of exposure. The quantity of dye employed will vary with the specific dye or dye combination chosen as well as the size and aspect ratio of the grains. It is known in the photographic art that optimum spectral sensitization is obtained with organic dyes at about 25 to 100 percent or more of monolayer coverage of the total available surface area of surface sensitive silver halide grains, as disclosed, for example, in West et al, "The Adsorption of Sensitizing Dyes in Photographic Emulsions", *Journal of Phys. Chem.*, Vol. 56, p. 1065, 1952; Spence et al, "Desensitization of Sensitizing Dyes," *Journal of Physical and Colloid Chemistry*, Vol. 56, No. 6, June 1948, pp. 1090-1103; and Gilman et al U.S. Pat. No. 3,979,213. Optimum dye concentration levels can be chosen by procedures taught by Mees, *Theory of the Photographic Process*, 60 1942, Macmillan, pp. 1067-1069.

Spectral sensitization can be undertaken at any stage of emulsion preparation heretofore known to be useful. Most commonly spectral sensitization is undertaken in the art subsequent to the completion of chemical sensitization. However, it is specifically recognized that spectral sensitization can be undertaken alternatively concurrent with chemical sensitization, can entirely precede chemical sensitization, and can even commence

prior to the completion of silver halide grain precipitation, as taught by Philippaerts et al U.S. Pat. No. 3,628,960, and Locker et al U.S. Pat. No. 4,225,666. As taught by Locker et al, it is specifically contemplated to distribute introduction of the spectral sensitizing dye into the emulsion so that a portion of the spectral sensitizing dye is present prior to chemical sensitization and a remaining portion is introduced after chemical sensitization. Unlike Locker et al, it is specifically contemplated that the spectral sensitizing dye can be added to the emulsion after 80 percent of the silver halide has been precipitated. Sensitization can be enhanced by pAg adjustment, including cycling, during chemical and/or spectral sensitization. A specific example of pAg adjustment is provided by *Research Disclosure*, Vol. 181, 15 May 1979, Item 18155.

Maskasky U.S. Ser. No. 431,855, filed concurrently herewith and commonly assigned, titled *CONTROLLED SITE EPITAXIAL SENSITIZATION*, which is a continuation-in-part of U.S. Ser. No. 320,920, filed Nov. 12, 1981, now abandoned, both here incorporated by reference, discloses the chemical sensitization of spectrally sensitized high aspect ratio tabular grain emulsions at one or more ordered discrete edge sites of the tabular grains. It is believed that the preferential absorption of spectral sensitizing dye on the crystallographic surfaces forming the major faces of the tabular grains allows chemical sensitization to occur selectively at unlike crystallographic surfaces along the edges and preferably at the corners of the tabular grains.

Although not required to realize all of their advantages, the emulsions of the present invention are preferably, in accordance with prevailing manufacturing practices, substantially optimally chemically and spectrally sensitized. That is, they preferably achieve speeds of at least 60 percent of the maximum log speed attainable from the grains in the spectral region of sensitization under the contemplated conditions of use and processing. Log speed is herein defined as 100 (1-log E), where E is measured in meter-candle-seconds at a density of 0.1 above fog. Once the silver halide grains of an emulsion have been characterized it is possible to estimate from further product analysis and performance evaluation whether an emulsion layer of a product appears to be substantially optimally chemically and spectrally sensitized in relation to comparable commercial offerings of other manufacturers. To achieve the sharpness advantages of the present invention it is immaterial whether the silver halide emulsions are chemically or spectrally sensitized efficiently or inefficiently.

Once high aspect ratio tabular grain emulsions have been generated by precipitation procedures, washed, and sensitized, as described above, their preparation can be completed by the incorporation of conventional photographic addenda, and they can be usefully applied to photographic applications requiring a silver image to be produced—e.g., conventional black-and-white photography.

Dickerson U.S. Ser. No. 430,574, filed concurrently herewith and commonly assigned, titled *FOREHARDENED PHOTOGRAPHIC ELEMENTS AND PROCESSES FOR THEIR USE*, which is a continuation-in-part of U.S. Ser. No. 320,910, filed Nov. 12, 1981, now abandoned, both here incorporated by reference, discloses that hardening photographic elements according to the present invention intended to form silver images to an extent sufficient to obviate the necessity of incorporating additional hardener during processing permits

increased silver covering power to be realized as compared to photographic elements similarly hardened and processed, but employing nontabular or less than high aspect ratio tabular grain emulsions. Specifically, it is taught to harden the high aspect ratio tabular grain emulsion layers and other hydrophilic colloid layers of black-and-white photographic elements in an amount sufficient to reduce swelling of the layers to less than 200 percent, percent swelling being determined by (a) incubating the photographic element at 38° C. for 3 days at 50 percent relative humidity, (b) measuring layer thickness, (c) immersing the photographic element in distilled water at 21° C. for 3 minutes, and (d) measuring change in layer thickness. Although hardening of the photographic elements intended to form silver images to the extent that hardeners need not be incorporated in processing solutions is specifically preferred, it is recognized that the emulsions of the present invention can be hardened to any conventional level. It is further specifically contemplated to incorporate hardeners in processing solutions, as illustrated, for example, by *Research Disclosure*, Vol. 184, August 1979, Item 18431, Paragraph K, relating particularly to the processing of radiographic materials.

Typical useful incorporated hardeners (forehardeners) include formaldehyde and free dialdehydes, such as succinaldehyde and glutaraldehyde, as illustrated by Allen et al U.S. Pat. No. 3,232,764; blocked dialdehydes, as illustrated by Kaszuba U.S. Pat. No. 2,586,168, Jeffreys U.S. Pat. No. 2,870,013, and Yamamoto et al U.S. Pat. No. 3,819,608;  $\alpha$ -diketones, as illustrated by Allen et al U.S. Pat. No. 2,725,305; active esters of the type described by Burness et al U.S. Pat. No. 3,542,558; sulfonate esters, as illustrated by Allen et al U.S. Pat. Nos. 2,725,305 and 2,726,162; active halogen compounds, as illustrated by Burness U.S. Pat. No. 3,106,468, Silverman et al U.S. Pat. No. 3,839,042, Ballantine et al U.S. Pat. No. 3,951,940 and Himmelmann et al U.S. Pat. No. 3,174,861; s-triazines and diazines, as illustrated by Yamamoto et al U.S. Pat. No. 3,325,287, Anderau et al U.S. Pat. No. 3,288,775 and Stauner et al U.S. Pat. No. 3,992,366; epoxides, as illustrated by Allen et al U.S. Pat. No. 3,047,394, Burness U.S. Pat. No. 3,189,459 and Birr et al German Pat. No. 1,085,663; aziridines, as illustrated by Allen et al U.S. Pat. No. 2,950,197, Burness et al U.S. Pat. No. 3,271,175 and Sata et al U.S. Pat. No. 3,575,705; active olefins having two or more active vinyl groups (e.g. vinylsulfonyl groups), as illustrated by Burness et al U.S. Pat. Nos. 3,490,911, 3,539,644 and 3,841,872 (Reissue 29,305), Cohen U.S. Pat. No. 3,640,720, Kleist et al German Pat. No. 872,153 and Allen U.S. Pat. No. 2,992,109; blocked active olefins, as illustrated by Burness et al U.S. Pat. No. 3,360,372 and Wilson U.S. Pat. No. 3,345,177; carbodiimides, as illustrated by Blout et al German Pat. No. 1,148,446; isoxazolium salts unsubstituted in the 3-position, as illustrated by Burness et al U.S. Pat. No. 3,321,313; esters of 2-alkoxy-N-carboxydihydroquinoline, as illustrated by Bergthaller et al U.S. Pat. No. 4,013,468; N-carbamoyl and N-carbamoyloxy-pyridinium salts, as illustrated by Himmelmann U.S. Pat. No. 3,880,665; hardeners of mixed function, such as halogen-substituted aldehyde acids (e.g., mucochloric and mucobromic acids), as illustrated by White U.S. Pat. No. 2,080,019, 'onium substituted acroleins, as illustrated by Tschopp et al U.S. Pat. No. 3,792,021, and vinyl sulfones containing other hardening functional groups, as illustrated by Sera et al U.S. Pat. No.

4,028,320; and polymeric hardeners, such as dialdehyde starches, as illustrated by Jeffreys et al U.S. Pat. No. 3,057,723, and copoly(acrolein-methacrylic acid), as illustrated by Himelmann et al U.S. Pat. No. 3,396,029.

The use of forehardeners in combination is illustrated by Sieg et al U.S. Pat. No. 3,497,358, Dallon et al U.S. Pat. No. 3,832,181 and 3,840,370 and Yamamoto et al U.S. Pat. No. 3,898,089. Hardening accelerators can be used, as illustrated by Sheppard et al U.S. Pat. No. 2,165,421, Kleist German Pat. No. 881,444, Riebel et al U.S. Pat. No. 3,628,961 and Ugi et al U.S. Pat. No. 3,901,708. The patents illustrative of hardeners and hardener combinations are here incorporated by reference.

Instability which increases minimum density in negative type emulsion coatings (i.e., fog) or which increases minimum density or decreases maximum density in direct-positive emulsion coatings can be protected against by incorporation of stabilizers, antifoggants, antikinking agents, latent image stabilizers and similar addenda in the emulsion and contiguous layers prior to coating. Many of the antifoggants which are effective in emulsions can also be used in developers and can be classified under a few general headings, as illustrated by C. E. K. Mees, *The Theory of the Photographic Process*, 2nd Ed., Macmillan, 1954, pp. 677-680.

To avoid such instability in emulsion coatings stabilizers and antifoggants can be employed, such as halide ions (e.g., chloride salts); chloropalladates and chloropalladates, as illustrated by Trivelli et al U.S. Pat. No. 2,566,263; water-soluble inorganic salts of magnesium, calcium, cadmium, cobalt, manganese and zinc, as illustrated by Jones U.S. Pat. No. 2,839,405 Sidebotham U.S. Pat. No. 3,488,709; mercury salts, as illustrated by Allen et al U.S. Pat. No. 2,728,663; selenols and diselenides, as illustrated by Brown et al U.K. Pat. No. 1,336,570 and Pollet et al U.K. Pat. No. 1,282,303; quaternary ammonium salts of the type illustrated by Allen et al U.S. Pat. No. 2,694,716, Brooker et al U.S. Pat. No. 2,131,038, Graham U.S. Pat. No. 3,342,596 and Arai et al U.S. Pat. No. 3,954,478; azomethine desensitizing dyes, as illustrated by Thiers et al U.S. Pat. No. 3,630,744; isothiourea derivatives, as illustrated by Herz et al U.S. Pat. No. 3,220,839 and Knott et al U.S. Pat. No. 2,514,650; thiadiazolidines, as illustrated by Scavron U.S. Pat. No. 3,565,625; peptide derivatives, as illustrated by Maffet U.S. Pat. No. 3,274,002; pyrimidines and 3-pyrazolidones, as illustrated by Welsh U.S. Pat. No. 3,161,515 and Hood et al U.S. Pat. No. 2,751,297; azotriazoles and azotetrazoles, as illustrated by Baldassari et al U.S. Pat. No. 3,925,086; azaindenes, particularly tetraazaindenes, as illustrated by Heimbach U.S. Pat. No. 2,444,605, Knott U.S. Pat. No. 2,933,388, Williams U.S. Pat. No. 3,202,512, *Research Disclosure*, Vol. 134, June 1975, Item 13452, and Vol. 148, August 1976, Item 14851, and Nepker et al U.K. Pat. No. 1,338,567; mercaptotetrazoles, -triazoles and -diazoles, as illustrated by Kendall et al U.S. Pat. No. 2,403,927, Kennard et al U.S. Pat. No. 3,266,897, *Research Disclosure*, Vol. 116, December 1973, Item 11684, Luckey et al U.S. Pat. No. 3,397,987 and Salesin U.S. Pat. No. 3,708,303; azoles, as illustrated by Peterson et al U.S. Pat. No. 2,271,229 and *Research Disclosure*, Item 11684, cited above; purines, as illustrated by Sheppard et al U.S. Pat. No. 2,319,090, Birr et al U.S. Pat. No. 2,152,460, *Research Disclosure*, Item 13452, cited above, and Dostes et al French Pat. No. 2,296,204 and polymers of 1,3-dihydroxy(and/or 1,3-carbamoxy)-2-

methylenepropane, as illustrated by Saleck et al U.S. Pat. No. 3,926,635.

Among useful stabilizers for gold sensitized emulsions are water-insoluble gold compounds of benzothiazole, benzoxazole, naphthothiazole and certain merocyanine and cyanine dyes, as illustrated by Yutzy et al U.S. Pat. No. 2,597,915, and sulfinamides, as illustrated by Nishio et al U.S. Pat. No. 3,498,792.

Among useful stabilizers in layers containing poly(alkylene oxides) are tetraazaindenes, particularly in combination with Group VIII noble metals or resorcinol derivatives, as illustrated by Carroll et al U.S. Pat. No. 2,716,062, U.K. Pat. No. 1,466,024 and Habu et al U.S. Pat. No. 3,929,486; quaternary ammonium salts of the type illustrated by Piper U.S. Pat. No. 2,886,437; water-insoluble hydroxides, as illustrated by Maffet U.S. Pat. No. 2,953,455; phenols, as illustrated by Smith U.S. Pat. Nos. 2,955,037 and '038; ethylene diurea, as illustrated by Dersch U.S. Pat. No. 3,582,346; barbituric acid derivatives, as illustrated by Wood U.S. Pat. No. 3,617,290; boranes, as illustrated by Bigelow U.S. Pat. No. 3,725,078; 3-pyrazolidinones, as illustrated by Wood U.K. Pat. No. 1,158,059 and aldoximines, amides, anilides and esters, as illustrated by Butler et al U.K. Pat. No. 988,052.

The emulsions can be protected from fog and desensitization caused by trace amounts of metals such as copper, lead, tin, iron and the like, by incorporating addenda, such as sulfocatechol-type compounds, as illustrated by Kennard et al U.S. Pat. No. 3,236,652; aldoximines, as illustrated by Carroll et al U.K. Pat. No. 623,448 and meta- and poly-phosphates, as illustrated by Draisbach U.S. Pat. No. 2,239,284, and carboxylic acids such as ethylenediamine tetraacetic acid, as illustrated by U.K. Pat. No. 691,715.

Among stabilizers useful in layers containing synthetic polymers of the type employed as vehicles and to improve covering power are monohydric and polyhydric phenols, as illustrated by Forsgard U.S. Pat. No. 3,043,697; saccharides, as illustrated by U.K. Pat. No. 897,497 and Stevens et al U.K. Pat. No. 1,039,471 and quinoline derivatives, as illustrated by Dersch et al U.S. Pat. No. 3,446,618.

Among stabilizers useful in protecting the emulsion layers against dichroic fog are addenda, such as salts of nitron, as illustrated by Barbier et al U.S. Pat. Nos. 3,679,424 and 3,820,998; mercaptocarboxylic acids, as illustrated by Willems et al U.S. Pat. No. 3,600,178, and addenda listed by E. J. Birr, *Stabilization of Photographic Silver Halide Emulsions*, Focal Press, London, 1974, pp. 126-218.

Among stabilizers useful in protecting emulsion layers against development fog are addenda such as azabenzimidazoles, as illustrated by Bloom et al U.K. Pat. No. 1,356,142 and U.S. Pat. No. 3,575,699, Rogers U.S. Pat. No. 3,473,924 and Carlson et al U.S. Pat. No. 3,649,267; substituted benzimidazoles, benzothiazoles, benzotriazoles and the like, as illustrated by Brooker et al U.S. Pat. No. 2,131,038, Land U.S. Pat. No. 2,704,721, Rogers et al U.S. Pat. No. 3,265,498; mercapto-substituted compounds, e.g., mercaptotetrazoles, as illustrated by Dimsdale et al U.S. Pat. No. 2,432,864, Rauch et al U.S. Pat. No. 3,081,170, Weyerts et al U.S. Pat. No. 3,260,597, Grasshoff et al U.S. Pat. No. 3,674,478 and Arond U.S. Pat. No. 3,706,557; isothiourea derivatives, as illustrated by Herz et al U.S. Pat. No. 3,220,839, and thiadiazole derivatives, as illustrated

by von Konig U.S. Pat. No. 3,364,028 and von Konig et al U.K. Pat. No. 1,186,441.

Where hardeners of the aldehyde type are employed, the emulsion layers can be protected with antifoggants, such as monohydric and polyhydric phenols of the type illustrated by Sheppard et al U.S. Pat. No. 2,165,421; nitro-substituted compounds of the type disclosed by Rees et al U.K. Pat. No. 1,269,268; poly(alkylene oxides), as illustrated by Valbusa U.K. Pat. No. 1,151,914, and mucohalogenic acids in combination with urazoles, as illustrated by Allen et al U.S. Pat. Nos. 3,232,761 and 3,232,764, or further in combination with maleic acid hydrazide, as illustrated by Rees et al U.S. Pat. No. 3,295,980.

To protect emulsion layers coated on linear polyester supports addenda can be employed such as parabanic acid, hydantoin acid hydrazides and urazoles, as illustrated by Anderson et al U.S. Pat. No. 3,287,135, and piazines containing two symmetrically fused 6-member carbocyclic rings, especially in combination with an aldehyde-type hardening agent, as illustrated in Rees et al U.S. Pat. No. 3,396,023.

Kink desensitization of the emulsions can be reduced by the incorporation of thallous nitrate, as illustrated by Overman U.S. Pat. No. 2,628,167; compounds, polymeric latices and dispersions of the type disclosed by Jones et al U.S. Pat. Nos. 2,759,821 and '822; azole and mercaptotetrazole hydrophilic colloid dispersions of the type disclosed by *Research Disclosure*, Vol. 116, December 1973, Item 11684; plasticized gelatin compositions of the type disclosed by Milton et al U.S. Pat. No. 3,033,680; water-soluble interpolymers of the type disclosed by Rees et al U.S. Pat. No. 3,536,491; polymeric latices prepared by emulsion polymerization in the presence of poly(alkylene oxide), as disclosed by Pearson et al U.S. Pat. No. 3,772,032, and gelatin graft copolymers of the type disclosed by Rakoczy U.S. Pat. No. 3,837,861.

Where the photographic element is to be processed at elevated bath or drying temperatures, as in rapid access processors, pressure desensitization and/or increased fog can be controlled by selected combinations of addenda, vehicles, hardeners and/or processing conditions, as illustrated by Abbott et al U.S. Pat. No. 3,295,976, Barnes et al U.S. Pat. No. 3,545,971, Salesin U.S. Pat. No. 3,708,303, Yamamoto et al U.S. Pat. No. 3,615,619, Brown et al U.S. Pat. No. 3,623,873, Taber U.S. Pat. No. 3,671,258, Abele U.S. Pat. No. 3,791,830, *Research Disclosure*, Vol. 99, July 1972, Item 9930, Florens et al U.S. Pat. No. 3,843,364, Priem et al U.S. Pat. No. 3,867,152, Adachi et al U.S. Pat. No. 3,967,965 and Mikawa et al U.S. Pat. Nos. 3,947,274 and 3,954,474.

In addition to increasing the pH or decreasing the pAg of an emulsion and adding gelatin, which are known to retard latent image fading, latent image stabilizers can be incorporated, such as amino acids, as illustrated by Ezekiel U.K. Pat. Nos. 1,335,923, 1,378,354, 1,387,654 and 1,391,672, Ezekiel et al U.K. Pat. No. 1,394,371, Jefferson U.S. Pat. No. 3,843,372, Jefferson et al U.K. Pat. No. 1,412,294 and Thurston U.K. Pat. No. 1,343,904; carbonyl-bisulfite addition products in combination with hydroxybenzene or aromatic amine developing agents, as illustrated by Seiter et al U.S. Pat. No. 3,424,583; cycloalkyl-1,3-diones, as illustrated by Beckett et al U.S. Pat. No. 3,447,926; enzymes of the catalase type, as illustrated by Matejec et al U.S. Pat. No. 3,600,182; halogen-substituted hardeners in combination with certain cyanine dyes, as illustrated by Kumai et al

U.S. Pat. No. 3,881,933; hydrazides, as illustrated by Honig et al U.S. Pat. No. 3,386,831; alkenylbenzothiazolium salts, as illustrated by Arai et al U.S. Pat. No. 3,954,478; soluble and sparingly soluble mercaptides, as illustrated by Herz U.S. Pat. No. 4,374,196, commonly assigned and here incorporated by reference; hydroxy-substituted benzylidene derivatives, as illustrated by Thurston U.K. Pat. No. 1,308,777 and Ezekiel et al U.K. Pat. Nos. 1,347,544 and 1,353,527; mercapto-substituted compounds of the type disclosed by Sutherns U.S. Pat. No. 3,519,427; metal-organic complexes of the type disclosed by Matejec et al U.S. Pat. No. 3,639,128; penicillin derivatives, as illustrated by Ezekiel U.K. Pat. No. 1,389,089; propynylthio derivatives of benzimidazoles, pyrimidines, etc., as illustrated by von Konig et al U.S. Pat. No. 3,910,791; combinations of iridium and rhodium compounds, as disclosed by Yamasue et al U.S. Pat. No. 3,901,713; sydrones or sydnone imines, as illustrated by Noda et al U.S. Pat. No. 3,881,939; thiazolidine derivatives, as illustrated by Ezekiel U.K. Pat. No. 1,458,197 and thioether-substituted imidazoles, as illustrated by *Research Disclosure*, Vol. 136, August 1975, Item 13651.

In addition to sensitizers, hardeners, and antifoggants and stabilizers, a variety of other conventional photographic addenda can be present. The specific choice of addenda depends upon the exact nature of the photographic application and is well within the capability of the art. A variety of useful addenda are disclosed in *Research Disclosure*, Vol. 176, December 1978, Item 17643, here incorporated by reference. Optical brighteners can be introduced, as disclosed by Item 17643 at Paragraph V. Absorbing and scattering materials can be employed in the emulsions of the invention and in separate layers of the photographic elements, as described in Paragraph VIII. Coating aids, as described in Paragraph XI, and plasticizers and lubricants, as described in Paragraph XII, can be present. Antistatic layers, as described in Paragraph XIII, can be present. Methods of addition of addenda are described in Paragraph XIV. Matting agents can be incorporated, as described in Paragraph XVI. Developing agents and development modifiers can, if desired, be incorporated, as described in Paragraphs XX and XXI. When the photographic elements of the invention are intended to serve radiographic applications, emulsion and other layers of the radiographic element can take any of the forms specifically described in *Research Disclosure*, Item 18431, cited above, here incorporated by reference. The emulsions of the invention, as well as other, conventional silver halide emulsion layers, interlayers, overcoats, and subbing layers, if any, present in the photographic elements can be coated and dried as described in Item 17643, Paragraph XV.

In accordance with established practices within the art it is specifically contemplated to blend the high aspect ratio tabular grain emulsions of the present invention with each other or with conventional emulsions to satisfy specific emulsion layer requirements. For example, it is known to blend emulsions to adjust the characteristic curve of a photographic element to satisfy a predetermined aim. Blending can be employed to increase or decrease maximum densities realized on exposure and processing, to decrease or increase minimum density, and to adjust characteristic curve shape intermediate its toe and shoulder. To accomplish this the emulsions of this invention can be blended with

conventional silver halide emulsions, such as those described in Item 17643, cited above, Paragraph I.

In their simplest form photographic elements according to the present invention employ a single emulsion layer containing a high aspect ratio tubular grain silver chloride emulsion according to the present invention and a photographic support. It is, of course, recognized that more than one silver halide emulsion layer as well as overcoat, subbing, and interlayers can be usefully included. Instead of blending emulsions as described above the same effect can usually be achieved by coating the emulsions to be blended as separate layers. Coating of separate emulsion layers to achieve exposure latitude is well known in the art, as illustrated by Zelikman and Levi, *Making and Coating Photographic Emulsions*, Focal Press, 1964, pp. 234-238; Wyckoff U.S. Pat. No. 3,663,228; and U.K. Pat. No. 923,045. It is further well known in the art that increased photographic speed can be realized when faster and slower emulsions are coated in separate layers as opposed to blending. Typically the faster emulsion layer is coated to lie nearer the exposing radiation source than the slower emulsion layer. This approach can be extended to three or more superimposed emulsion layers. Such layer arrangements are specifically contemplated in the practice of this invention.

The layers of the photographic elements can be coated on a variety of supports. Typical photographic supports include polymeric film, wood fiber—e.g., paper, metallic sheet and foil, glass and ceramic supporting elements provided with one or more subbing layers to enhance the adhesive, antistatic, dimensional, abrasive, hardness, frictional, antihalation and/or other properties of the support surface.

Typical of useful polymeric film supports are films of cellulose nitrate and cellulose esters such as cellulose triacetate and diacetate, polystyrene, polyamides, homo- and co-polymers of vinyl chloride, poly(vinyl acetal), polycarbonate, homo- and co-polymers of olefins, such as polyethylene and polypropylene, and polyesters of dibasic aromatic carboxylic acids with divalent alcohols, such as poly(ethylene terephthalate).

Typical of useful paper supports are those which are partially acetylated or coated with baryta and/or a polyolefin, particularly a polymer of an  $\alpha$ -olefin containing 2 to 10 carbon atoms, such as polyethylene, polypropylene, copolymers of ethylene and propylene and the like.

Polyolefins, such as polyethylene, polypropylene and polyallomers—e.g., copolymers of ethylene with propylene, as illustrated by Hagemeyer et al U.S. Pat. No. 3,478,128, are preferably employed as resin coatings over paper, as illustrated by Crawford et al U.S. Pat. No. 3,411,908 and Joseph et al U.S. Pat. No. 3,630,740, over polystyrene and polyester film supports, as illustrated by Crawford et al U.S. Pat. No. 3,630,742, or can be employed as unitary flexible reflection supports, as illustrated by Venor et al U.S. Pat. No. 3,973,963.

Preferred cellulose ester supports are cellulose triacetate supports, as illustrated by Fordyce et al U.S. Pat. Nos. 2,492,977, '978 and 2,739,069, as well as mixed cellulose ester supports, such as cellulose acetate propionate and cellulose acetate butyrate, as illustrated by Fordyce et al U.S. Pat. No. 2,739,070.

Preferred polyester film supports are comprised of linear polyester, such as illustrated by Alles et al U.S. Pat. No. 2,627,088, Wellman U.S. Pat. No. 2,720,503, Alles U.S. Pat. No. 2,779,684 and Kibler et al U.S. Pat.

No. 2,901,466. Polyester films can be formed by varied techniques, as illustrated by Alles, cited above, Czerkas et al U.S. Pat. No. 3,663,683 and Williams et al U.S. Pat. No. 3,504,075, and modified for use as photographic film supports, as illustrated by Van Stappen U.S. Pat. No. 3,227,576, Nadeau et al U.S. Pat. No. 3,501,301, Reedy et al U.S. Pat. No. 3,589,905, Babbitt et al U.S. Pat. No. 3,850,640, Baily et al U.S. Pat. No. 3,888,678, Hunter U.S. Pat. No. 3,904,420 and Mallinson et al U.S. Pat. No. 3,928,697.

The photographic elements can employ supports which are resistant to dimensional change at elevated temperatures. Such supports can be comprised of linear condensation polymers which have glass transition temperatures above about 190° C., preferably 220° C., such as polycarbonates, polycarboxylic esters, polyamides, polysulfonamides, polyethers, polyimides, polysulfonates and copolymer variants, as illustrated by Hamb U.S. Pat. Nos. 3,634,089 and 3,772,405; Hamb et al U.S. Pat. Nos. 3,725,070 and 3,793,249; Wilson *Research Disclosure*, Vol. 118, February 1974, Item 11833, and Vol. 120, April 1974, Item 12046; Conklin et al *Research Disclosure*, Vol. 120, April 1974, Item 12012; Product Licensing Index, Vol. 92, December 1971, Items 9205 and 9207; *Research Disclosure*, Vol. 101, September 1972, Items 10119 and 10148; *Research Disclosure*, Vol. 106, February 1973, Item 10613; *Research Disclosure*, Vol. 117, January 1974, Item 11709, and *Research Disclosure*, Vol. 134, June 1975, Item 13455.

Although the emulsion layer or layers are typically coated as continuous layers on supports having opposed planar major surfaces, this need not be the case. The emulsion layers can be coated as laterally displaced layer segments on a planar support surface. When the emulsion layer or layers are segmented, it is preferred to employ a microcellular support. Useful microcellular supports are disclosed by Whitmore Patent Cooperation Treaty published application W080/01614, published August 7, 1980, (Belgian Pat. No. 881,513, August 1, 1980, corresponding), Blazey et al U.S. Pat. No. 4,307,165, and Gilmour et al U.S. Ser. No. 293,080, filed August 17, 1981, here incorporated by reference. Microcells can range from 1 to 200 microns in width and up to 1000 microns in depth. It is generally preferred that the microcells be at least 4 microns in width and less than 200 microns in depth, with optimum dimensions being about 10 to 100 microns in width and depth for ordinary black-and-white imaging applications—particularly where the photographic image is intended to be enlarged.

The photographic elements of the present invention can be imagewise exposed in any conventional manner. Attention is directed to *Research Disclosure* Item 17643, cited above, Paragraph XVIII, here incorporated by reference. The present invention is particularly advantageous when imagewise exposure is undertaken with electromagnetic radiation within the region of the spectrum in which the spectral sensitizers present exhibit absorption maxima. When the photographic elements are intended to record blue, green, red, or infrared exposures, spectral sensitizer absorbing in the blue, green, red, or infrared portion of the spectrum is present. For black-and-white imaging applications it is preferred that the photographic elements be orthochromatically or panchromatically sensitized to permit light to extend sensitivity within the visible spectrum. Radiant energy employed for exposure can be either noncoherent (random phase) or coherent (in phase),

produced by lasers. Imagewise exposures at ambient, elevated or reduced temperatures and/or pressures, including high or low intensity exposures, continuous or intermittent exposures, exposure times ranging from minutes to relatively short durations in the millisecond to microsecond range and solarizing exposures, can be employed within the useful response ranges determined by conventional sensitometric techniques, as illustrated by T. H. James, *The Theory of the Photographic Process*, 4th Ed., Macmillan, 1977, Chapters 4, 6, 17, 18, and 23.

The light-sensitive silver halide contained in the photographic elements can be processed following exposure to form a visible image by associating the silver halide with an aqueous alkaline medium in the presence of a developing agent contained in the medium or the element. Processing formulations and techniques are described in L. F. Mason, *Photographic Processing Chemistry*, Focal Press, London, 1966; *Processing Chemicals and Formulas*, Publication J-1, Eastman Kodak Company, 1973; *Photo-Lab Index*, Morgan and Morgan, Inc., Dobbs Ferry, New York, 1977, and *Nebblette's Handbook of Photography and Reprography-Materials, Processes and Systems*, VanNostrand Reinhold Company, 7th Ed., 1977.

Included among the processing methods are web processing, as illustrated by Tregillus et al U.S. Pat. No. 3,179,517; stabilization processing, as illustrated by Herz et al U.S. Pat. No. 3,220,839, Cole U.S. Pat. No. 3,615,511, Shipton et al U.K. Pat. No. 1,258,906 and Haist et al U.S. Pat. No. 3,647,453; monobath processing as described in Haist, *Monobath Manual*, Morgan and Morgan, Inc., 1966, Shuler U.S. Pat. No. 3,240,603, Haist et al U.S. Pat. Nos. 3,615,513 and 3,628,955 and Price U.S. Pat. No. 3,723,126; infectious development, as illustrated by Milton U.S. Pat. Nos. 3,294,537, 3,600,174, 3,615,519 and 3,615,524, Whiteley U.S. Pat. No. 3,516,830, Drago U.S. Pat. No. 3,615,488, Salesin et al U.S. Pat. No. 3,625,689, Illingsworth U.S. Pat. No. 3,632,340, Salesin U.K. Pat. No. 1,273,030 and U.S. Pat. No. 3,708,303; hardening development, as illustrated by Allen et al U.S. Pat. No. 3,232,761; roller transport processing, as illustrated by Russell et al U.S. Pat. Nos. 3,025,779 and 3,515,556, Masseth U.S. Pat. No. 3,573,914, Taber et al U.S. Pat. No. 3,647,459 and Rees et al U.K. Pat. No. 1,269,268; alkaline vapor processing, as illustrated by *Product Licensing Index*, Vol. 97, May 1972, Item 9711, Goffe et al U.S. Pat. No. 3,816,136 and King U.S. Pat. No. 3,985,564; metal ion development as illustrated by Price, *Photographic Science and Engineering*, Vol. 19, Number 5, 1975, pp. 283-287 and Vought 50 *Research Disclosure*, Vol. 150, October 1976; Item 15034; reversal processing, as illustrated by Henn et al U.S. Pat. No. 3,576,633; and surface application processing, as illustrated by Kitze U.S. Pat. No. 3,418,132.

Once a silver image has been formed in the photographic element, it is conventional practice to fix the undeveloped silver halide. The high aspect ratio tubular grain emulsions of the present invention are particularly advantageous in allowing fixing to be accomplished in a shorter time period. This allows processing to be accelerated.

The photographic elements and the techniques described above for producing silver images can be readily adapted to provide a colored image through the use of dyes. In perhaps the simplest approach to obtaining a projectable color image a conventional dye can be incorporated in the support of the photographic element, and silver image formation undertaken as de-

scribed above. In areas where a silver image is formed the element is rendered substantially incapable of transmitting light therethrough, and in the remaining areas light is transmitted corresponding in color to the color of the support. In this way a colored image can be readily formed. The same effect can also be achieved by using a separate dye filter layer or element with a transparent support element.

The silver halide photographic elements can be used to form dye images therein through the selective destruction or formation of dyes. The photographic elements described above for forming silver images can be used to form dye images by employing developers containing dye image formers, such as color couplers, as illustrated by U.K. Pat. No. 478,984, Yager et al U.S. Pat. No. 3,113,864, Vittum et al U.S. Pat. Nos. 3,002,836, 2,271,238 and 2,362,598, Schwan et al U.S. Pat. No. 2,950,970, Carroll et al U.S. Pat. No. 2,592,243, Porter et al U.S. Pat. Nos. 2,343,703, 2,376,380 and 2,369,489, Spath U.K. Pat. No. 886,723 and U.S. Pat. No. 2,899,306, Tuite U.S. Pat. No. 3,152,896 and Mannes et al U.S. Pat. Nos. 2,115,394, 2,252,718 and 2,108,602, and Pilato U.S. Pat. No. 3,547,650. In this form the developer contains a color-developing agent (e.g., a primary aromatic amine) which in its oxidized form is capable of reacting with the coupler (coupling) to form the image dye.

The dye-forming couplers can be incorporated in the photographic elements, as illustrated by Schneider et al, *Die Chemie*, Vol. 57, 1944, p. 113, Mannes et al U.S. Pat. No. 2,304,940, Martinez U.S. Pat. No. 2,269,158, Jelley et al U.S. Pat. No. 2,322,027, Frolich et al U.S. Pat. No. 2,376,679, Fierke et al U.S. Pat. No. 2,801,171, Smith U.S. Pat. No. 3,748,141, Tong U.S. Pat. No. 2,772,163, Thirtle et al U.S. Pat. No. 2,835,579, Sawdey et al U.S. Pat. No. 2,533,514, Peterson U.S. Pat. No. 2,353,754, Seidel U.S. Pat. No. 3,409,435 and Chen Research Disclosure, Vol. 159, July 1977, Item 15930. The dye-forming couplers can be incorporated in different amounts to achieve differing photographic effects. For example, U.K. Pat. No. 923,045 and Kumai et al U.S. Pat. No. 3,843,369 teach limiting the concentration of coupler in relation to the silver coverage to less than normally employed amounts in faster and intermediate speed emulsion layers.

The dye-forming couplers are commonly chosen to form subtractive primary (i.e., yellow, magenta and cyan) image dyes and are nondiffusible, colorless couplers, such as two and four equivalent couplers of the open chain ketomethylene, pyrazolone, pyrazolotriazole, pyrazolobenzimidazole, phenol and naphthol type hydrophobically ballasted for incorporation in high-boiling organic (coupler) solvents. Such couplers are illustrated by Salminen et al U.S. Pat. Nos. 2,423,730, 2,772,162, 2,895,826, 2,710,803, 2,407,207, 3,737,316 and 2,367,531, Loria et al U.S. Pat. Nos. 2,772,161, 2,600,788, 3,006,759, 3,214,437 and 3,253,924, McCrossen et al U.S. Pat. No. 2,875,057, Bush et al U.S. Pat. No. 2,908,573, Gledhill et al U.S. Pat. No. 3,034,892, Weissberger et al U.S. Pat. Nos. 2,474,293, 2,407,210, 3,062,653, 3,265,506 and 3,384,657, Porter et al U.S. Pat. No. 2,343,703, Greenhalgh et al U.S. Pat. No. 3,127,269, Feniak et al U.S. Pat. No. 2,865,748, 2,933,391 and 2,865,751, Bailey et al U.S. Pat. No. 3,725,067, Beavers et al U.S. Pat. No. 3,758,308, Lau U.S. Pat. No. 3,779,763, Fernandez U.S. Pat. No. 3,785,829, U.K. Pat. No. 969,921, U.K. Pat. No. 1,241,069, U.K. Pat. No. 1,011,940, Vanden Eynde et al

U.S. Pat. No. 3,762,921, Beavers U.S. Pat. No. 2,983,608, Loria U.S. Pat. Nos. 3,311,476, 3,408,194, 3,458,315, 3,447,928, 3,476,563, Cressman et al U.S. Pat. No. 3,419,390, Young U.S. Pat. No. 3,419,391, Lestina U.S. Pat. No. 3,519,429, U.K. Pat. No. 975,928, U.K. Pat. No. 1,111,554, Jaeken U.S. Pat. No. 3,222,176 and Canadian Pat. No. 726,651, Schulte et al U.K. Pat. No. 1,248,924 and Whitmore et al U.S. Pat. No. 3,227,550. Dye-forming couplers of differing reaction rates in single or separate layers can be employed to achieve desired effects for specific photographic applications.

The dye-forming couplers upon coupling can release photographically useful fragments, such as development inhibitors or accelerators, bleach accelerators, developing agents, silver halide solvents, toners, hardeners, fogging agents, antifogants, competing couplers, chemical or spectral sensitizers and desensitizers. Development inhibitor-releasing (DIR) couplers are illustrated by Whitmore et al U.S. Pat. No. 3,148,062, Barr et al U.S. Pat. No. 3,227,554, Barr U.S. Pat. No. 3,733,201, Sawdye U.S. Pat. No. 3,617,291, Groet et al U.S. Pat. No. 3,703,375, Abbott et al U.S. Pat. No. 3,615,506, Weissberger et al U.S. Pat. No. 3,265,506, Seymour U.S. Pat. No. 3,620,745, Marx et al U.S. Pat. No. 3,632,345, Mader et al U.S. Pat. No. 3,869,291, U.K. Pat. No. 1,201,110, Oishi et al U.S. Pat. No. 3,642,485, Verbrugge, U.K. Pat. No. 1,236,767, Fujiwhara et al U.S. Pat. No. 3,770,436 and Matsuo et al U.S. Pat. No. 3,808,945. Dye-forming couplers and nondye-forming compounds which upon coupling release a variety of photographically useful groups are described by Lau U.S. Pat. No. 4,248,962. DIR compounds which do not form dye upon reaction with oxidized color-developing agents can be employed, as illustrated by Fujiwhara et al German OLS 2,529,350 and U.S. Pat. Nos. 3,928,041, 3,958,993 and 3,961,959, Odenwalder et al German OLS No. 2,448,063, Tanaka et al German OLS No. 2,610,546, Kikuchi et al U.S. Pat. No. 4,049,455 and Credner et al U.S. Pat. No. 4,052,213. DIR compounds which oxidatively cleave can be employed, as illustrated by Porter et al U.S. Pat. No. 3,379,529, Green et al U.S. Pat. No. 3,043,690, Barr U.S. Pat. No. 3,364,022, Duennebier et al U.S. Pat. No. 3,297,445 and Rees et al U.S. Pat. No. 3,287,129. Silver halide emulsions which are relatively light insensitive, such as Lipmann emulsions, having been utilized as interlayers and overcoat layers to prevent or control the migration of development inhibitor fragments as described in Shiba et al U.S. Pat. No. 3,892,572.

The photographic elements can incorporate colored dye-forming couplers, such as those employed to form integral masks for negative color images, as illustrated by Hanson U.S. Pat. No. 2,449,966, Glass et al U.S. Pat. No. 2,521,908, Gledhill et al U.S. Pat. No. 3,034,892, Loria U.S. Pat. No. 3,476,563, Lestina U.S. Pat. No. 3,519,429, Friedman U.S. Pat. No. 2,543,691, Puschel et al U.S. Pat. No. 3,028,238, Menzel et al U.S. Pat. No. 3,061,432 and Greenhalgh U.K. Pat. No. 1,035,959, and/or competing couplers, as illustrated by Murin et al U.S. Pat. No. 3,876,428, Sakamoto et al U.S. Pat. No. 3,580,722, Puschel U.S. Pat. No. 2,998,314, Whitmore U.S. Pat. No. 2,808,329, Salminen U.S. Pat. No. 2,742,832 and Weller et al U.S. Pat. No. 2,689,793.

The photographic elements can include image dye stabilizers. Such image dye stabilizers are illustrated by U.K. Pat. No. 1,326,889, Lestina et al U.S. Pat. Nos. 3,432,300 and 3,698,909, Stern et al U.S. Pat. No. 3,574,627, Brannock et al U.S. Pat. No. 3,573,050, Arai

et al U.S. Pat. No. 3,764,337 and Smith et al U.S. Pat. No. 4,042,394.

Dye images can be formed or amplified by processes which employ in combination with a dye-image-generating reducing agent an inert transition metal ion complex oxidizing agent, as illustrated by Bissonette U.S. Pat. Nos. 3,748,138, 3,826,652, 3,862,842 and 3,989,526 and Travis U.S. Pat. No. 3,765,891, and/or a peroxide oxidizing agent, as illustrated by Matejec U.S. Pat. No. 3,674,490, *Research Disclosure*, Vol. 116, December 1973, Item 11660, and Bissonette *Research Disclosure*, Vol. 148, August 1976, Items 14836, 14846 and 14847. The photographic elements can be particularly adapted to form dye images by such processes, as illustrated by Dunn et al U.S. Pat. No. 3,822,129, Bissonette U.S. Pat. Nos. 3,834,907 and 3,902,905, Bissonette et al U.S. Pat. No. 3,847,619 and Mowrey U.S. Pat. No. 3,904,413.

The photographic elements can produce dye images through the selective destruction of dyes or dye precursors, such as silver-dye-bleach processes, as illustrated by A. Meyer, *The Journal of Photographic Science*, Vol. 13, 1965, pp. 90-97. Bleachable azo, azoxy, xanthene, azine, phenylmethane, nitroso complex, indigo, quinone, nitro-substituted, phthalocyanine and formazan dyes, as illustrated by Stauner et al U.S. Pat. No. 3,754,923, Piller et al U.S. Pat. No. 3,749,576, Yoshida et al U.S. Pat. No. 3,738,839, Froelich et al U.S. Pat. No. 3,716,368, Piller U.S. Pat. No. 3,655,388, Williams et al U.S. Pat. No. 3,642,482, Gilman U.S. Pat. No. 3,567,448, Loeffel U.S. Pat. No. 3,443,953, Anderau U.S. Pat. Nos. 3,443,952 and 3,211,556, Mory et al U.S. Pat. Nos. 3,202,511 and 3,178,291 and Anderau et al U.S. Pat. Nos. 3,178,285 and 3,178,290, as well as their hydrazo, diazonium and tetrazonium precursors and leuco and shifted derivatives, as illustrated by U.K. Pat. Nos. 923,265, 999,996 and 1,042,300, Pelz et al U.S. Pat. No. 3,684,513, Watanabe et al U.S. Pat. No. 3,165,493, Wilson et al U.S. Pat. No. 3,503,741, Boes et al U.S. Pat. No. 3,340,059, Gompf et al U.S. Pat. No. 3,493,372 and Puschel et al U.S. Pat. No. 3,561,970, can be employed.

It is common practice in forming dye images in silver halide photographic elements to remove the developed silver by bleaching. Such removal can be enhanced by incorporation of a bleach accelerator or a precursor thereof in a processing solution or in a layer of the element. In some instances the amount of silver formed by development is small in relation to the amount of dye produced, particularly in dye image amplification, as described above, and silver bleaching is omitted without substantial visual effect. In still other applications the silver image is retained and the dye image is intended to enhance or supplement the density provided by the image silver. In the case of dye enhanced silver imaging it is usually preferred to form a neutral dye or a combination of dyes which together produce a neutral image. Neutral dye-forming couplers useful for this purpose are disclosed by Pupo et al *Research Disclosure*, Vol. 162, October 1977, Item 16226. The enhancement of silver images with dyes in photographic elements intended for thermal processing is disclosed in *Research Disclosure*, Vol. 173, September 1973, Item 17326 and Houle U.S. Pat. No. 4,137,079. It is also possible to form monochromatic or neutral dye images using only dyes, silver being entirely removed from the image-bearing photographic elements by bleaching and fixing, as illustrated by Marchant et al U.S. Pat. No. 3,620,747.

The photographic elements can be processed to form dye images which correspond to or are reversals of the silver halide rendered selectively developable by imagewise exposure. Reversal dye images can be formed in photographic elements having differentially spectrally sensitized silver halide layers by black-and-white development followed by (i) where the elements lack incorporated dye image formers, sequential reversal color development with developers containing dye image formers, such as color couplers, as illustrated by 10 Mannes et al U.S. Pat. No. 2,252,718, Schwan et al U.S. Pat. No. 2,950,970 and Pilato U.S. Pat. No. 3,547,650; (ii) where the elements contain incorporated dye image formers, such as color couplers, a single color development step, as illustrated by the Kodak Ektachrome E4 15 and E6 and Agfa processes described in *British Journal of Photography Annual*, 1977, pp. 194-197, and *British Journal of Photography*, August 2, 1974, pp. 668-669; and (iii) where the photographic elements contain bleachable dyes, silver-dye-bleach processing, as illustrated by the Cibachrome, P-10 and P-18 processes described in the *British Journal of Photography Annual*, 1977, pp. 209-212.

The photographic elements can be adapted for direct color reversal processing (i.e., production of reversal 25 color images without prior black-and-white development), as illustrated by U.K. Pat. No. 1,075,385, Barr U.S. Pat. No. 3,243,294, Hendess et al U.S. Pat. No. 3,647,452, Puschel et al German Pat. No. 1,257,570 and U.S. Pat. Nos. 3,457,077 and 3,467,520, Accary-Venet et al U.K. Pat. No. 1,132,736, Schranz et al German Pat. No. 1,259,700, Marx et al German Pat. No. 1,259,701 and Muller-Bore German OLS 2,005,091.

Dye images which correspond to the silver halide rendered selectively developable by imagewise exposure, typically negative dye images, can be produced by processing, as illustrated by the Kodacolor C-22, the Kodak Flexicolor C-41 and the Agfacolor processes described in *British Journal of Photography Annual*, 1977, pp. 201-205. The photographic elements can also 35 be processed by the Kodak Ektaprint-3 and -300 processes as described in Kodak Color Dataguide, 5th Ed., 1975, pp. 18-19, and the Agfa color process as described in *British Journal of Photography Annual*, 1977, pp. 205-206, such processes being particularly suited to 40 processing color print materials, such as resin-coated photographic papers, to form positive dye images.

The present invention can be employed to produce multicolor photographic images, as taught by Kofron et al, cited above. Generally any conventional multicolor 50 imaging element containing at least one silver halide emulsion layer can be improved merely by adding or substituting a high aspect ratio tabular grain emulsion according to the present invention. The present invention is fully applicable to both additive multicolor imaging and subtractive multicolor imaging.

To illustrate the application of this invention to additive multicolor imaging, a filter array containing interlaid blue, green, and red filter elements can be employed in combination with a photographic element according 60 to the present invention capable of producing a silver image. A high aspect ratio tabular grain emulsion of the present invention which is panchromatically sensitized and which forms a layer of the photographic element is imagewise exposed through the additive primary filter array. After processing to produce a silver image and viewing through the filter array, a multicolor image is seen. Such images are best viewed by projection. Hence

both the photographic element and the filter array both have or share in common a transparent support.

Significant advantages can be realized by the application of this invention to multicolor photographic elements which produce multicolor images from combinations of subtractive primary imaging dyes. Such photographic elements are comprised of a support and typically at least a triad of superimposed silver halide emulsion layers for separately recording blue, green, and red exposures as yellow, magenta, and cyan dye images, respectively.

Although only one high aspect ratio tabular grain silver chloride emulsion as described above is required, the multicolor photographic element contains at least three separate emulsions for recording blue, green, and red light, respectively. The emulsions other than the required high aspect ratio tabular grain green or red recording emulsion can be of any convenient conventional form. Various conventional emulsions are illustrated by *Research Disclosure*, Item 17643, cited above, Paragraph I, Emulsion preparation and types, here incorporated by reference. If more than one emulsion layer is provided to record in the blue, green, and/or red portion of the spectrum, it is preferred that at least the faster emulsion layer contain a high aspect ratio tabular grain emulsion as described above. It is, of course, recognized that all of the blue, green, and red recording emulsion layers of the photographic element can advantageously be tabular grain emulsions according to this invention, if desired.

Multicolor photographic elements are often described in terms of color-forming layer units. Most commonly multicolor photographic elements contain three superimposed color-forming layer units each containing at least one silver halide emulsion layer capable of recording exposure to a different third of the spectrum and capable of producing a complementary subtractive primary dye image. Thus, blue, green, and red recording color-forming layer units are used to produce yellow, magenta, and cyan dye images, respectively. Dye imaging materials need not be present in any color-forming layer unit, but can be entirely supplied from processing solutions. When dye imaging materials are incorporated in the photographic element, they can be located in an emulsion layer or in a layer located to receive oxidized developing or electron transfer agent from an adjacent emulsion layer of the same color-forming layer unit.

To prevent migration of oxidized developing or electron transfer agents between color-forming layer units with resultant color degradation, it is common practice to employ scavengers. The scavengers can be located in the emulsion layers themselves, as taught by Yutzy et al U.S. Pat. No. 2,937,086 and/or in interlayers containing scavengers are provided between adjacent color-forming layer units, as illustrated by Weissberger et al U.S. Pat. No. 2,336,327.

Although each color-forming layer unit can contain a single emulsion layer, two, three, or more emulsion layers differing in photographic speed are often incorporated in a single color-forming layer unit. Where the desired layer order arrangement does not permit multiple emulsion layers differing in speed to occur in a single color-forming layer unit, it is common practice to provide multiple (usually two or three) blue, green, and/or red recording color-forming layer units in a single photographic element.

The multicolor photographic elements can take any convenient form consistent with the requirements indicated above. Any of the six possible layer arrangements of Table 27a, p. 211, disclosed by Gorokhovskii, *Spectral Studies of the Photographic Process*, Focal Press, New York, can be employed. To provide a simple, specific illustration, it is contemplated to add to a conventional multicolor silver halide photographic element during its preparation one or more high aspect ratio tabular grain emulsion layers sensitized to the minus blue portion of the spectrum and positioned to receive exposing radiation prior to the remaining emulsion layers. However, in most instances it is preferred to substitute one or more minus blue recording high aspect ratio tabular grain emulsion layers for conventional minus blue recording emulsion layers, optionally in combination with layer order arrangement modifications. Alternative layer arrangements can be better appreciated by reference to following preferred illustrative forms.

| Layer Order Arrangement I |   |
|---------------------------|---|
| Exposure                  | ↓ |
| ↓                         | B |
| IL                        |   |
| TG                        |   |
| IL                        |   |
| TR                        |   |

  

| Layer Order Arrangement II |     |
|----------------------------|-----|
| Exposure                   | ↓   |
| ↓                          | TFB |
| TFB                        | IL  |
| IL                         | TFG |
| TFG                        | IL  |
| IL                         | TFR |
| TFR                        | IL  |
| IL                         | SB  |
| SB                         | IL  |
| IL                         | SG  |
| SG                         | IL  |
| IL                         | SR  |

  

| Layer Order Arrangement III |    |
|-----------------------------|----|
| Exposure                    | ↓  |
| ↓                           | TG |
| TG                          | IL |
| IL                          | TR |
| TR                          | IL |
| IL                          | B  |

  

| Layer Order Arrangement IV |     |
|----------------------------|-----|
| Exposure                   | ↓   |
| ↓                          | TFG |
| TFG                        | IL  |
| IL                         | TFR |
| TFR                        | IL  |
| IL                         | TSG |
| TSG                        | IL  |
| IL                         | TSR |
| TSR                        | IL  |
| IL                         | B   |

  

| Layer Order Arrangement V |     |
|---------------------------|-----|
| Exposure                  | ↓   |
| ↓                         | TFG |
| TFG                       | IL  |
| IL                        | TFR |
| TFR                       | IL  |
| IL                        | TFB |
| TFB                       | IL  |
| IL                        | TSG |
| TSG                       | IL  |
| IL                        | TSR |
| TSR                       | IL  |
| IL                        | SB  |

where

B, G, and R designate blue, green, and red recording color-forming layer units, respectively, of any conventional type;

5 T appearing before the color-forming layer unit B, G, or R indicates that the emulsion layer or layers contain a high aspect ratio tabular grain silver chloride emulsion, as more specifically described above;

F appearing before the color-forming layer unit B, G, 10 or R indicates that the color-forming layer unit is faster in photographic speed than at least one other color-forming layer unit which records light exposure in the same third of the spectrum in the same Layer Order Arrangement;

S appearing before the color-forming layer unit B, G, 15 or R indicates that the color-forming layer unit is slower in photographic speed than at least one other color-forming layer unit which records light exposure in the same third of the spectrum in the same Layer Order Arrangement; and

20 IL designates an interlayer containing a scavenger, but substantially free of yellow filter material. Each faster or slower color-forming layer unit can differ in photographic speed from another color-forming layer

25 unit which records light exposure in the same third of the spectrum as a result of its position in the Layer Order Arrangement, its inherent speed properties, or a combination of both.

In Layer Order Arrangements I through V, the location 30 of the support is not shown. Following customary practice, the support will in most instances be positioned farthest from the source of exposing radiation—that is, beneath the layers as shown. If the support is colorless and specularly transmissive—i.e., transparent, 35 it can be located between the exposure source and the indicated layers. Stated more generally, the support can be located between the exposure source and any color-forming layer unit intended to record light to which the support is transparent.

40 Although photographic emulsions intended to form multicolor images comprised of combinations of subtractive primary dyes normally take the form of a plurality of superimposed layers containing incorporated dye-forming materials, such as dye-forming couplers, 45 this is by no means required. Three color-forming components, normally referred to as packets, each containing a silver halide emulsion for recording light in one third of the visible spectrum and a coupler capable of forming a complementary subtractive primary dye, can

50 be placed together in a single layer of a photographic element to produce multicolor images. Exemplary mixed packet multicolor photographic elements are disclosed by Godowsky U.S. Pat. Nos. 2,698,794 and 2,843,489. Although discussion is directed to the more 55 common arrangement in which a single color-forming layer unit produces a single subtractive primary dye, relevance to mixed packet multicolor photographic elements will be readily apparent.

As described by Kofron et al, cited above, the high 60 aspect ratio tabular grain silver bromoiodide emulsions of the present invention are advantageous because of their reduced high angle light scattering as compared to nontabular and lower aspect ratio tabular grain emulsions. This can be quantitatively demonstrated. Referring 65 to FIG. 5, a sample of an emulsion 1 according to the present invention is coated on a transparent (specularly transmissive) support 3 at a silver coverage of 1.08 g/m<sup>2</sup>. Although not shown, the emulsion and support

are preferably immersed in a liquid having a substantially matched refractive index to minimize Fresnel reflections at the surfaces of the support and the emulsion. The emulsion coating is exposed perpendicular to the support plane by a collimated light source 5. Light from the source following a path indicated by the dashed line 7, which forms an optical axis, strikes the emulsion coating at point A. Light which passes through the support and emulsion can be sensed at a constant distance from the emulsion at a hemispherical detection surface 9. At a point B, which lies at the intersection of the extension of the initial light path and the detection surface, light of a maximum intensity level is detected.

An arbitrarily selected point C is shown in FIG. 5 on the detection surface. The dashed line between A and C forms an angle  $\phi$  with the emulsion coating. By moving point C on the detection surface it is possible to vary  $\phi$  from  $0^\circ$  to  $90^\circ$ . By measuring the intensity of the light scattered as a function of the angle  $\phi$  it is possible (because of the rotational symmetry of light scattering about the optical axis 7) to determine the cumulative light distribution as a function of the angle  $\phi$ . (For a background description of the cumulative light distribution see DePalma and Gasper, "Determining the Optical Properties of Photographic Emulsions by the Monte Carlo Method," *Photographic Science and Engineering*, Vol. 16, No. 3, May-June 1971, pp. 181-191.)

After determining the cumulative light distribution as a function of the angle  $\phi$  at values from  $0^\circ$  to  $90^\circ$  for the emulsion 1 according to the present invention, the same procedure is repeated, but with a conventional emulsion of the same average grain volume coated at the same silver coverage on another portion of support 3. In comparing the cumulative light distribution as a function of the angle  $\phi$  for the two emulsions, for values of  $\phi$  up to  $70^\circ$  (and in some instances up to  $80^\circ$  and higher) the amount of scattered light is lower with the emulsions according to the present invention. Thus, the high aspect ratio tabular grain emulsions of this invention exhibit less high-angle scattering. Since it is high-angle scattering of light that contributes disproportionately to reduction in image sharpness, it follows that the high aspect ratio tabular grain emulsions of the present invention are in each instance capable of producing sharper images.

In FIG. 5 the angle  $\phi$  is shown as the complement of the angle  $\phi$ . As herein defined the term "collection angle" is the value of the angle  $\phi$  at which half of the light striking the detection surface lies within an area subtended by a cone formed by rotation of line AC about the polar axis at the angle  $\phi$  while half of the light striking the detection surface strikes the detection surface within the remaining area.

While not wishing to be bound by any particular theory to account for the reduced high angle scattering properties of high aspect ratio tabular grain emulsions according to the present invention, it is believed that the large flat major crystal faces presented by the high aspect ratio tabular grains as well as the orientation of the grains in the coating account for the improvements in sharpness observed. Specifically, it has been observed that the tabular grains present in a silver halide emulsion coating are substantially aligned with the planar support surface on which they lie. Thus, light directed perpendicular to the photographic element striking the emulsion layer tends to strike the tabular grains substantially perpendicular to one major crystal face. The thinness of

5 tabular grains as well as their orientation when coated permits the high aspect ratio tabular grain emulsion layers of this invention to be substantially thinner than conventional emulsion coatings, which can also contribute to sharpness. However, the emulsion layers of this invention exhibit enhanced sharpness even when they are coated to the same thicknesses as conventional emulsion layers.

In a specific preferred form of the invention the high aspect ratio tabular grain emulsion layers exhibit a minimum average grain diameter of at least 1.0 micron, most preferably at least 2 microns. Both improved speed and sharpness are attainable as average grain diameters are increased. While maximum useful average grain diameters will vary with the graininess that can be tolerated for a specific imaging application, the maximum average grain diameters of high aspect ratio tabular grain emulsions according to the present invention are in all instances less than 30 microns, preferably less than 15 microns, and optimally no greater than 10 microns.

20 Although it is possible to obtain reduced high angle scattering with single layer coatings of high aspect ratio tabular grain emulsions according to the present invention, it does not follow that reduced high angle scattering is necessarily realized in multicolor coatings. In certain multicolor coating formats enhanced sharpness can be achieved with the high aspect ratio tabular grain emulsions of this invention, but in other multicolor coating formats the high aspect ratio tabular grain emulsions of this invention can actually degrade the sharpness of underlying emulsion layers.

25 Referring back to Layer Order Arrangement I, it can be seen that the blue recording emulsion layer lies nearest to the exposing radiation source while the underlying green recording emulsion layer is a tabular grain emulsion according to this invention. The green recording emulsion layer in turn overlies the red recording emulsion layer. If the blue recording emulsion layer contains grains having an average diameter in the range of from 0.2 to 0.6 micron, as is typical of many nontabular emulsions, it will exhibit maximum scattering of light passing through it to reach the green and red recording emulsion layers. Unfortunately, if light has already been scattered before it reaches the high aspect ratio tabular grain emulsion forming the green recording emulsion layer, the tabular grains can scatter the light passing through to the red recording emulsion layer to an even greater degree than a conventional emulsion. Thus, this particular choice of emulsions and layer arrangement results in the sharpness of the red recording emulsion layer being significantly degraded to an extent greater than would be the case if no emulsions according to this invention were present in the layer order arrangement.

30 In order to realize fully the sharpness advantages in an emulsion layer that underlies a high aspect ratio tabular grain silver chloride emulsion layer according to the present invention it is preferred that the tabular grain emulsion layer be positioned to receive light that is free of significant scattering. Stated another way, improvements in sharpness in emulsion layers underlying tabular grain emulsion layers are best realized only when the tabular grain emulsion layer does not itself underlie a turbid layer. For example, if a high aspect ratio tabular grain green recording emulsion layer overlies a red recording emulsion layer and underlies a Lippmann emulsion layer and/or a high aspect ratio tabular grain blue recording emulsion layer according to this invention, the sharpness of the red recording emulsion

layer will be improved by the presence of the overlying tabular grain emulsion layer or layers. Stated in quantitative terms, if the collection angle of the layer or layers overlying the high aspect ratio tabular grain green recording emulsion layer is less than about 10°, an improvement in the sharpness of the red recording emulsion layer can be realized. It is, of course, immaterial whether the red recording emulsion layer is itself a high aspect ratio tabular grain emulsion layer according to this invention insofar as the effect of the overlying layers on its sharpness is concerned.

In a multicolor photographic element containing superimposed color-forming units it is preferred that at least the emulsion layer lying nearest the source of exposing radiation be a high aspect ratio tabular grain emulsion in order to obtain the advantages of sharpness. In a specifically preferred form each emulsion layer which lies nearer the exposing radiation source than another image recording emulsion layer is a high aspect ratio tabular grain emulsion layer. Layer Order Arrangements II, III, IV, and V, described above, are illustrative of multicolor photographic element layer arrangements which are capable of imparting significant increases in sharpness to underlying emulsion layers.

Although the advantageous contribution of high aspect ratio tabular grain silver chloride emulsions to image sharpness in multicolor photographic elements has been specifically described by reference to multicolor photographic elements, sharpness advantages can also be realized in multilayer black-and-white photographic elements intended to produce silver images. It is conventional practice to divide emulsions forming black-and-white images into faster and slower layers. By employing high aspect ratio tabular grain emulsions according to this invention in layers nearest the exposing radiation source the sharpness of underlying emulsion layers will be improved.

#### EXAMPLES

The invention can be better appreciated by reference to the following specific examples.

In each of the examples the contents of the reaction vessel were stirred vigorously throughout silver and halide salt introductions; the term "percent" means percent by weight, unless otherwise indicated; and all solutions, unless otherwise indicated, are aqueous solutions.

#### EXAMPLE 1

Tabular grain AgCl emulsion prepared at 30° C.

A 2.0 liter aqueous bone gelatin solution (2.0% gelatin 0.001 N NH<sub>4</sub>NO<sub>3</sub>, Solution A) was adjusted at 30° C. to pH 9.05 by adding a 7.5 N aqueous ammonium hydroxide solution (Solution D) and pCl 1.05 by adding an aqueous bone gelatin solution (4.2% gelatin) containing ammonium chloride (2.01 molar, Solution B). To Solution A, maintained at 30° C., pH 9.05 and pCl 1.05 (pAg 8.5), were added by double-jet addition at constant flow rate for 5 minutes (6.7% of total silver consumed), Solution B and an aqueous solution of silver nitrate (2.00 molar, Solution C).

After the initial 5 minute period, Solutions B and C were added by double-jet addition at an accelerated flow rate (6× from start to finish—i.e., six times faster at the end than at the start) while maintaining pCl 1.05 and 30° C. (approximately 20 minutes, consuming 93.3% of total silver used). Simultaneously, a third jet was used to

add Solution D at a rate sufficient to maintain pH 9.05. 4.5 Moles of silver were used to prepare this emulsion. In each of the examples the contents of the reaction vessel were stirred vigorously throughout silver and halide salt introductions.

A tabular AgCl emulsion prepared by this procedure is shown in FIG. 1. (The photomicrograph was taken at 1000× magnification). More than 50 percent of the projected areas of the silver chloride grains is in the form of tabular grains. The tabular grains are less than 0.6 micron in thickness and exhibit an average aspect ratio of approximately 10:1.

#### EXAMPLE 2

15 Tabular grain AgCl emulsion prepared at 40° C. A 1.0 liter aqueous bone gelatin solution (6% gelatin, 0.1 N NH<sub>4</sub>NO<sub>3</sub>, Solution A) was adjusted at 40° C. to pH 8.8 by adding a 3.75 N aqueous ammonium hydroxide solution (Solution D) and pCl 1.3 by adding an aqueous ammonium chloride (2.00 molar)/ammonium hydroxide (0.2 N) solution (Solution B). To Solution A, maintained at 40° C. and pCl 1.3 (pAg 7.9), were added by double-jet addition at constant flow rate, Solution B and an aqueous silver nitrate solution (2.00 molar, Solution C) until Solution C ran out (approximately 25 minutes). Simultaneously, Solution D was added via a third jet to Solution A at a rate sufficient to maintain pH 8.8. 1.0 Mole of silver was used to prepare this emulsion.

20 A tabular grain AgCl emulsion prepared by this procedure is shown in FIG. 2. (The photomicrograph was taken at 500× magnification). There are a higher proportion (greater than 50 percent projected area) of tabular silver chloride grains in the emulsion of FIG. 2 than in FIG. 1. The average aspect ratio of the tabular grains is approximately 10:1.

#### EXAMPLE 3

Tabular grain AgCl emulsion prepared at 60° C.

25 A 1.0 liter aqueous bone gelatin solution (8% gelatin, Solution A) was adjusted at 60° C. to pH 8.8 by adding a 7.5 N aqueous ammonium hydroxide solution (Solution D) and pCl 1.3 (pAg 7.3) by adding an aqueous ammonium chloride (2.00 molar)/ammonium hydroxide (0.2 N) solution (Solution B). To Solution A, while maintaining 60° C. and pCl 1.3 were added by double-jet addition at a constant flow rate, Solution B and an aqueous silver nitrate solution (2.00 molar, Solution C) until Solution C was depleted (approximately 25 minutes). Simultaneously, Solution D was added to Solution A at a rate sufficient to maintain pH 8.8. 1.0 Mole of silver was used to prepare this emulsion.

30 A tabular grain AgCl emulsion prepared by this procedure is shown in FIG. 3. (The photomicrograph was taken at 250× magnification). More than 75 percent of the total projected area of the silver chloride grains in FIG. 3 are tabular. The tabular silver chloride grains have an average aspect ratio of greater than 10:1.

#### EXAMPLE 4 (A COMPARATIVE EXAMPLE)

35 Tabular grain AgCl emulsion prepared from 300 A AgI seed grains.

A 1.0 liter aqueous bone gelatin solution (6.0% gelatin, 0.1 N NH<sub>4</sub>NO<sub>3</sub>, Solution A) was adjusted at 40° C. to pH 8.8 by adding a 3.75 N aqueous ammonium hydroxide solution (Solution D), to pCl 1.3 (pAg 7.9) by adding an aqueous ammonium chloride (2.00 molar)/ammonium hydroxide (0.2 N) solution (Solution B) and adding 300 A AgI seed grains ( $6.25 \times 10^{-4}$  mole).

To Solution A, maintained at 40° C. and pCl 1.3 were added by double-jet addition at constant flow rate, Solution B and an aqueous solution of silver nitrate (2.00 molar, Solution C) until Solution C was depleted (approximately 25 minutes). Simultaneously, Solution D was added via a triple-jet at a rate sufficient to maintain pH 8.8. 1.0 Mole of silver was used to prepare this emulsion.

A tabular grain AgClI emulsion prepared by this example is shown in FIG. 4. (The photomicrograph was taken at 500 $\times$  magnification). The tabular silver chloroiodide grains of FIG. 4 are smaller in size as compared to the tabular silver chloride grains of FIG. 2, which were prepared at the same temperature. Further, there is a higher proportion of nontabular grains in FIG. 4 than in FIG. 2.

#### EXAMPLE 5

A tabular grain AgCl emulsion was prepared as described for Example 2, except 3.0 liters of a 4.0% gelatin solution were used, run time was for 16 minutes, 7.5 molar ammonium hydroxide was used to maintain pH, and a total of 3 moles of emulsion were precipitated. Following precipitation 1.0 liter of an aqueous gelatin (12.0 percent by weight) solution was added and the emulsion was washed by the coagulation process of Yutzy and Russell U.S. Pat. No. 2,614,929. Then 45 g. of bone gelatin was added and the emulsion was adjusted to pH 5.6 and pAg 7.5 at 40° C.

The resultant tabular grain AgCl emulsion had an average grain diameter of 6.3  $\mu$ m, an average grain thickness of 0.65  $\mu$ m, and an average aspect ratio of 9.7:1, and greater than 58% of the projected area was provided by the tabular grains.

The emulsion was chemically sensitized with 15 mg. gold sulfide/Ag mole and then coated on cellulose triacetate film support at 4.3 g. silver/m<sup>2</sup> and 12.9 g. gelatin/m<sup>2</sup>. The coating was exposed for 1 second to a 600 W 2850° K. tungsten light source through a 0-4.0 density continuous tablet and processed for 6 minutes in a N-methyl-p-aminophenol sulfate (Elon ®)-ascorbic acid surface developer at 20° C.

Sensitometric results revealed a significant negative image with a  $D_{min}$  of 0.10, a  $D_{max}$  of 0.90, and a contrast of 0.58.

The invention has been described in detail with particular reference to preferred embodiments thereof, but it will be understood that variations and modifications can be effected within the spirit and scope of the invention.

What is claimed is:

1. A radiation-sensitive photographic emulsion comprising a dispersing medium and silver chloride grains, wherein at least 50 percent of the total projected area of said silver chloride grains is provided by tabular grains which are substantially internally free of both bromide and iodide, have an average aspect ratio greater than 8:1, and have opposed, substantially parallel major {111} crystal faces.

2. A radiation-sensitive photographic emulsion according to claim 1, wherein at least 75 percent, based on total projected area, of said silver chloride grains is present in the form of tabular grains.

3. A radiation-sensitive photographic emulsion according to claim 1, wherein said tabular grains have an average aspect ratio of at least 10:1.

4. A radiation-sensitive photographic emulsion according to claim 1, wherein said tabular grains have an average thickness of less than 0.8 micron.

5. A radiation-sensitive photographic emulsion according to claim 1, wherein said dispersing medium contains gelatin or a gelatin derivative.

6. A radiation-sensitive photographic emulsion according to claim 1 wherein said tabular grains are of triangular or truncated triangular configuration.

7. In a photographic element comprised of a support and at least one radiation-sensitive emulsion layer, the improvement wherein said emulsion layer is comprised of an emulsion according to claim 1, 2, 3, 4, 5, or 6.

8. In a double-jet precipitation process of preparing a radiation-sensitive photographic emulsion comprised of a dispersing medium and silver halide grains which are substantially internally free of iodide and bromide by concurrently introducing chloride and silver salt solutions into the dispersing medium in the presence of ammonia,

the improvement comprising, while introducing the chloride salt solution,  
maintaining the pAg within the dispersing medium in the range of from 6.5 to 10 and  
maintaining the pH within the dispersing medium in the range of from 8 to 10,  
thereby precipitating at least 50 percent, based on total grain projected area, of the silver chloride grains in the form of tabular grains having an average aspect ratio greater than 8:1 and having opposed, substantially parallel major {111} crystal faces of triangular or truncated triangular configuration.

9. In an improved double-jet precipitation process according to claim 8, maintaining the pAg within the dispersing medium in the range of from 7.0 to 9.4.

10. In an improved double-jet precipitation process according to claim 8, maintaining the pH within the dispersing medium in the range of from 8.5 to 9.7.

11. In an improved double-jet precipitation process according to claim 8, maintaining the temperature of the reaction vessel below about 60° C.

12. In an improved double-jet precipitation process according to claim 11, maintaining the temperature of the reaction vessel in the range of from 20° to 40° C.

13. In an improved double-jet precipitation process according to claim 12, maintaining the pAg within in the range of from 7.6 to 8.9 and maintaining the pH in the range of from 8.8 to 9.5.

14. In an improved double-jet precipitation process according to claim 8 or 13, maintaining the pH within the dispersing medium by adding ammonium hydroxide to the reaction vessel concurrently with addition to the silver and chloride salt solutions.

15. In an improved double-jet precipitation process according to claim 14, employing a dispersing medium containing a peptizer.

16. In an improved double-jet precipitation process according to claim 15, employing gelatin or a gelatin derivative as the peptizer.

17. In an improved double-jet precipitation process according to claim 8 or 13, separating at least a portion of nontabular grains produced from the tabular silver chloride grains.

\* \* \* \* \*